



US005250407A

**United States Patent** [19]**Kase**[11] **Patent Number:** **5,250,407**[45] **Date of Patent:** **Oct. 5, 1993**

[54] **SILVER HALIDE COLOR PHOTOGRAPHIC LIGHT-SENSITIVE MATERIAL CONTAINING AT LEAST ONE 5-PYRAZOLONE COUPLER AND AT LEAST ONE MONODISPERSE CUBIC SILVER HALIDE EMULSION**

[75] Inventor: **Akira Kase, Kanagawa, Japan**

[73] Assignee: **Fuji Photo Film Co., Ltd., Kanagawa, Japan**

[21] Appl. No.: **834,981**

[22] Filed: **Feb. 14, 1992**

**Related U.S. Application Data**

[63] Continuation of Ser. No. 386,762, Jul. 31, 1989, abandoned.

**Foreign Application Priority Data**

Aug. 3, 1988 [JP] Japan ..... 63-193672

[51] Int. Cl.<sup>5</sup> ..... G03C 7/384; G03C 1/09  
[52] U.S. Cl. ..... 430/5.55; 430/567;  
430/569; 430/605

[58] **Field of Search** ..... 430/567, 569, 604, 605,  
430/555

**[56] References Cited****U.S. PATENT DOCUMENTS**

|           |         |                      |               |
|-----------|---------|----------------------|---------------|
| 3,854,949 | 12/1974 | Gilman, Jr. et al.   | ..... 430/567 |
| 4,248,962 | 2/1981  | Lau                  | ..... 430/382 |
| 4,269,927 | 5/1981  | Atwell               | ..... 430/604 |
| 4,741,994 | 5/1988  | Ichijima et al.      | ..... 430/549 |
| 4,746,603 | 5/1988  | Yamashita et al.     | ..... 430/605 |
| 4,842,994 | 7/1989  | Sakanoue et al.      | ..... 430/543 |
| 4,853,319 | 8/1989  | Krishnamurthy et al. | ..... 430/505 |
| 4,876,182 | 10/1989 | Buckland             | ..... 430/957 |
| 4,897,342 | 1/1990  | Kajiwara et al.      | ..... 430/605 |
| 4,900,657 | 2/1990  | Crawley et al.       | ..... 430/555 |
| 4,929,540 | 5/1990  | Furutuchi et al.     | ..... 430/555 |

**FOREIGN PATENT DOCUMENTS**

0194452 10/1985 Japan .

*Primary Examiner*—Lee C. Wright  
*Attorney, Agent, or Firm*—Birch, Stewart, Kolasch & Birch

**[57] ABSTRACT**

A silver halide color photographic light-sensitive material, comprising at least one silver halide light-sensitive emulsion layer provided on a support wherein at least one of said light-sensitive emulsion layer contains (i) at least one 5-pyrazolone coupler having an elimination group represented by the following general formula (I) at the coupling position thereof and (ii) at least one monodisperse cubic silver halide emulsion containing at least one metal ion selected from the group consisting of ions of metals of Group VIII of the Periodic Table, transition metals of Group II of the Periodic Table, lead and thallium in an amount of from  $1 \times 10^{-9}$  to  $1 \times 10^{-3}$  mol per mol of silver halide, said emulsion being obtained by incorporating said metal ion into silver halide grains in the silver halide light-sensitive emulsion by adding the ion to an emulsion formation system before or during formation of the grains or after formation of the grains but before the addition of a chemical sensitizer;

(I)

**14 Claims, No Drawings**

**SILVER HALIDE COLOR PHOTOGRAPHIC  
LIGHT-SENSITIVE MATERIAL CONTAINING AT  
LEAST ONE 5-PYRAZOLONE COUPLER AND AT  
LEAST ONE MONODISPERSE CUBIC SILVER  
HALIDE EMULSION**

This application is a continuation of application Ser. No. 07/386,762 filed on Jul. 31, 1989, now abandoned.

**FIELD OF THE INVENTION**

The present invention relates to a silver halide color photographic light-sensitive material and an image forming method using the same. More particularly, the present invention relates to a silver halide color photographic light-sensitive material which can be rapidly processed and is excellent in processing stability.

**BACKGROUND OF THE INVENTION**

A color photographic material which allows the processing time to be shortened and is not affected very much by processing factors is in demand. Also, a color photographic material having excellent stability during processing and an image forming method using such a color photographic material is in demand. Moreover, a color photographic material providing a short delivery time and a reduction in labor during the processing thereof has been in demand in recent years.

Methods for shortening the processing time in each processing stage include elevating the processing temperature or increasing the replenishment amount. Further, other methods have been proposed for shortening the processing time including, for example, methods wherein stirring is vigorously conducted and methods where various accelerators are added.

There are also known methods to attain a rapid color development and a reduced replenishment, wherein color photographic materials containing an emulsion are used having a high silver chloride content called a high silver chloride emulsion are used in the place of silver chlorobromide emulsions having a high silver bromide content which have been conventionally used. For example, WO87-04534 discloses a method for rapidly processing high silver chloride type silver halide color photographic materials by using color developing solutions containing substantially no sulfite ion or benzyl alcohol.

However, when color development is carried out according to the above method, there are problems including an insufficient rate of development, poor photographic sensitivity and a tendency of fogging when the developing time is prolonged in order to provide high sensitivity, even though the above method has a development accelerating effect as compared with conventional methods.

**SUMMARY OF THE INVENTION**

An object of the present invention is to provide a color photographic material which can be rapidly processed, is highly sensitive and has little fog over a wide exposure range, is not affected very much by fluctuations in development conditions and has a stable quality.

The above object of the present invention has been achieved by providing

(1) A silver halide color photographic light-sensitive material, comprising at least one silver halide light-sensitive emulsion layer provided on a support wherein at least one of said light-sensitive layers contains at least

one 5-pyrazolone coupler having an elimination group represented by the following general formula (I) at the coupling position thereof and at least one monodisperse cubic silver halide emulsion containing at least one metal ion selected from the group consisting of ions of metals of Group VIII of the Periodic Table, transition metals of Group II of the Periodic Table, lead and thallium in an amount of from  $1 \times 10^{-9}$  to  $1 \times 10^{-3}$  mol per mol of silver halide, which is incorporated into silver halide grains in the silver halide light-sensitive emulsion by adding the ion to an emulsion formation system before or during formation of the grains or after formation of the grains but before the addition of a chemical sensitizer;

(2) A silver halide color photographic light-sensitive material as in the preceding item (1), wherein a dry film thickness is not more than 15  $\mu\text{m}$  and a wet film thickness is from 20  $\mu\text{m}$  to 40  $\mu\text{m}$ ; and

(3) A method for forming an image of a silver halide color photograph, comprising processing the photographic material of the preceding item (1) or (2) by using a color developing solution containing chlorine ion in an amount of from  $3.5 \times 10^{-2}$  to  $1.5 \times 10^{-1}$  mol/l and bromine ion in an amount of from  $3.0 \times 10^{-5}$  to  $1.0 \times 10^{-3}$  mol/l.

The elimination group of general formula (I) is as follows:



wherein  $L_1$  and  $L_2$  each represents a methylene group or an ethylene group;  $l$  and  $m$  each represents 0 or 1;  $R^1$  represents a hydrogen atom, an alkyl group, an aryl group or a heterocyclic group;  $R_2$  represents a group linked with  $A$  and is a carbon atom, an oxygen atom, a nitrogen atom or a sulfur atom;  $A$  represents a carbon atom or a sulfur atom;  $n$  represents 1 when  $A$  is a carbon atom or  $n$  represents 1 or 2 when  $A$  is a sulfur atom;  $B$  represents a carbon atom, an oxygen atom, a nitrogen atom or a sulfur atom;  $X$  represents an atomic group required for the formation of a ring;  $R_1$  and  $R_2$  may be combined together to form a ring; and  $B$  and  $R_2$  may be combined together to form a ring when  $B$  is a carbon atom or a nitrogen atom.

**DETAILED DESCRIPTION OF THE  
INVENTION**

The present invention will be described in more detail hereinbelow.

With regard to the external form and the grain size of the silver halide emulsion of the present invention, cubic monodisperse silver halide emulsions are used.

The external forms of the silver halide grains can be observed through an electron microscope.

The cubic emulsion grains of the present invention include those in which the corners and edges of the cubes are almost round and they are apparently almost spheres. Emulsions containing quantitatively at least 50% of grains having a  $K$  value of preferably at least 7, more preferably at least 500, are used, wherein the  $K$

value is a ratio of (200) plane and (222) plane which constitute the outer surfaces of the silver halide grains.

The K value in the present invention is defined by the following formula:

$$K = \frac{\text{Intensity of diffraction line assigned to (200) plane}}{\text{Intensity of diffraction line assigned to (222) plane}}$$

The measurement of the intensity of the diffraction line in the present invention is described in, for example, *Bulletin of the Society of Scientific Photography of Japan*, Vol. 13, page 5. The intensity of the diffraction line can be determined by powder X-ray diffraction analysis of an emulsion containing silver halide grains oriented and coated on a substrate.

Preferably, the pyrazolone magenta couplers of the present invention are incorporated in monodisperse cubic silver halide emulsions containing a metal ion.

The silver halide of the present invention has a grain size of preferably not larger than 1.5  $\mu\text{m}$ , more preferably not larger than 1  $\mu\text{m}$ , but not smaller than 0.2  $\mu\text{m}$ .

The monodisperse silver halide grains of the present invention have such a grain size distribution that the ratio ( $S/\bar{r}$ ) of the standard deviation  $S$  to the mean grain size  $\bar{r}$  is preferably not higher than 0.2, and more preferably not higher than 0.15.

The grain size distribution and the mean grain size of the silver halide grains can be determined by measuring the projected areas of the silver halide grains from the electron micrograph and processing statistically the measured values according to the method described in T. H. James, *The Theory of the Photographic Process* (1977, Macmillan), Chapter 3, from page 100. With regard to the mean grain size, the arithmetical mean is used.

In this case, it is preferred that two or more of the above monodisperse emulsions are blended in the same layer or a multi-layer coating is conducted for the purpose of obtaining a wide latitude.

It is preferred that silver chloride or silver chlorobromide containing substantially no silver iodide is used as the halogen composition of the silver halide emulsion in the present invention. The term "containing substantially no silver iodide" as used herein means that the content of silver iodide is not higher than 1 mol %, preferably not higher than 0.2 mol %. The emulsion contains grains which may have the same or different halogen compositions. However, when an emulsion containing grains having the same halogen composition is used, the properties of the grains can be easily made homogeneous. With regard to the halogen composition distribution in the interior of the grains of the silver halide emulsion, there may be used any of the uniform structure type grains wherein the halogen composition is equal throughout the silver halide grains, laminated structure type grains wherein the core of the interior of the silver halide grain is different in halogen composition from a shell surrounding the core (including a single layer type as well as multi-layer type), and grains having such a structure that there exists areas having a different halogen composition in a non-laminar form in the interior of the grains or on the surfaces of grains (when there exist said areas on the surfaces of the grains, said areas having a different halogen composition are joined at the corners, edges or planes).

Preferably, from the viewpoint of pressure resistance, either of the latter two type of structures rather than an uniform structure type is used for the purpose of imparting high sensitivity. When silver halide grains having

the above-described structures are used, the boundary between areas having different halogen compositions may either be clear or unclear where a mixed crystal having difference in halogen composition is formed.

5 Alternatively, the boundary may have a continuous change in structure.

With regard to the halogen compositions of these silver chlorobromide emulsions, the ratio of silver bromide/silver chloride may be varied widely according to the intended purpose. Preferably, high silver chloride emulsions having a high silver chloride content are used for photographic materials suitable for use in rapid processing. These high silver chloride emulsions have a silver chloride content of preferably not lower than 90 mol %, more preferably not lower than 95 mol %.

10 Preferably, the high silver chloride emulsions have such a structure that silver bromide-localized phases exist in a laminar or non-laminar form in the interior portions of the silver halide grains and/or on the surfaces thereof.

15 Moreover, it is effective to further increase the silver chloride content of the silver halide emulsions for the purpose of reducing the replenishment rates of the developing solutions. In this case, approximately pure silver chloride emulsions having a silver chloride content of 98 to 100 mol % are preferred.

20 The localized phases preferably have such a halogen composition that the silver bromide content is at least 10 mol %, more preferably higher than 20 mol %. The localized phases are formed in the interior portions of grains or on the edges, corners or planes of the surfaces of the grains. In a preferred embodiment, localized phases are formed on the corners of the grains by epitaxial growth.

25 In some cases, uniform structure type grains having a narrow halogen composition distribution are preferred for the purpose of preventing the sensitivity from being lowered when pressure is applied to the photographic materials, even when high silver chloride emulsions having a silver chloride content of not lower than 90 mol % are used.

30 In the present invention, if there is no specific definition of the phase "metal ion", this phase means a metal ion or a metal complex ion which can be derived from a metal salt or a metal complex salt. The metal salt or metal complex salt may be an organic or inorganic metal salt or metal complex salt.

35 Examples of metal ions to be incorporated in the silver halide grains of the present invention include metal ions derived from Group VIII metals of the Periodic Table such as iron, iridium, platinum, palladium, nickel, rhodium, osmium, ruthenium and cobalt; Group II transition metals such as cadmium, zinc and mercury, and other metals such as lead, thallium and complex ions. At least one member of these metal ions or complex ions is used in the present invention. When silver halide grains have the above-mentioned localized phases, it is preferred that at least one of iridium ion, rhodium ion, iron ion are mainly used for the localized phases and a combination of metal ions selected from osmium, iridium, rhodium, platinum, ruthenium, palladium, cobalt, nickel and iron or complex ions thereof

40 are mainly used for the substrate. If desired, the localized phase and the substrate may be different in the type and concentration of the metal ions from each other. A plurality of the metal ions may be used.

Further, metal ions such as cadmium, zinc, lead, mercury and thallium ions can be used.

Now, these metal ions will be illustrated in more detail below.

Iridium ion-containing compounds are trivalent or tetravalent salts or complex salts. The complex salts are particularly preferred. Examples of the iridium ion-containing compounds include halide, amines and oxalato complex salts such as iridium(III) chloride, iridium(III) bromide, iridium (IV) chloride, sodium hexachloroiridate(III), potassium hexachloroiridate(IV), hexammineiridium(III) salt, trioxalatoiridate(III) and trioxalatoiridate(IV). These compounds are used in an amount preferably of  $5 \times 10^{-9}$  to  $1 \times 10^{-4}$  mol, more preferably from  $5 \times 10^{-8}$  to  $5 \times 10^{-6}$  mol per mol of silver.

Platinum ion-containing compounds are bivalent salts, tetravalent salts or complex salts, among which the complex salts are preferred. Examples of the platinum ion-containing compounds include platinum(IV) chloride, potassium hexachloroplatinate(IV), potassium tetrachloroplatinate(II), potassium tetrabromoplatinate(II), sodium tetrakis(thiocyanato)platinate(IV) and hexammineplatinum(IV) chloride. These compounds are used preferably in an amount of  $1 \times 10^{-8}$  to  $1 \times 10^{-5}$  mol per mol of silver.

Palladium ion-containing compounds are generally bivalent salts, tetravalent salts or complex salts, among which the complex salts are particularly preferred. Examples of the palladium ion-containing compounds include sodium tetrachloropalladate(II), sodium tetrachloropalladate(IV), potassium hexachloropalladate(IV), tetramminepalladium(II) chloride and potassium tetracyanopalladate(II).

Examples of nickel ion-containing compounds include nickel chloride, nickel bromide, potassium tetrachloronickelate(II), hexamminenickel(II) chloride and sodium tetracyanoniccolate(II).

Rhodium ion-containing compounds are preferably trivalent salts or complex salts. Examples thereof include potassium hexachlororhodate, sodium hexabromorhodate and ammonium hexachlororhodate. These compounds are used preferably in an amount of  $1 \times 10^{-8}$  to  $1 \times 10^{-4}$  mol per mol of silver.

Iron ion-containing compounds are ferric or ferrous compounds. Iron salts or complex salts which are water-soluble at a concentration to be used, are preferred. Iron complex salts which can be easily incorporated into silver halide grains are particularly preferred. Examples thereof include hexacyanoferrates (II), hexacyanoferrates(III), ferrous thiocyanate and ferric thiocyanate. These compounds are used preferably in an amount of  $5 \times 10^{-9}$  to  $1 \times 10^{-3}$  mol, more preferably  $1 \times 10^{-8}$  to  $1 \times 10^{-4}$  mol per mol of silver in silver halide.

The above-described metal ion donating compounds can be incorporated in the silver halide grains, for example, by adding the metal ion-donating compounds to an aqueous gelatin solution acting as a dispersion medium, an aqueous solution of a halide or an aqueous solution of a silver salt, or to another aqueous solution during the course of the formation of the silver halide grains. Alternatively, fine silver halide grains already containing metal ion therein are added to a host emulsion and dissolved thereto. The metal ion-donating compounds may be incorporated in the localized phases of silver halide grains and/or other parts (substrates).

The incorporation of the metal ion in the emulsion grains of the present invention can be carried out before, during or immediately after the formation of grains. The time when the metal ion is added, can be determined depending on the positions of the grains where the metal ion is to be located.

When the metal ion is added to the silver halide emulsion of the present invention, high sensitivity can be imparted thereto over a wide illumination intensity range. Particularly, when the photographic materials of the present invention are processed with color developing solutions containing chlorine ion in an amount of  $3.5 \times 10^{-2}$  to  $1.5 \times 10^{-1}$  mol/l and bromine ion in an amount of  $3.0 \times 10^{-5}$  to  $1.0 \times 10^{-3}$  mol/l, the materials of the present invention are characterized by low fogging and high sensitivity.

In addition to incorporation of the metal ion to the emulsion layer containing the 5-pyrazolone coupler of the present invention, the metal ion may also be added to any one of emulsion layers in the photographic material.

The silver halide emulsions of the present invention may be chemically sensitized. Examples of sensitization methods include a sulfur sensitization method using a sulfur compound capable of reacting with active gelatin or silver (e.g., thiosulfates, thioureas, mercapto compounds, rhodanines), a reduction sensitization method using a reducing material (e.g., stannous salts, amines, hydrazine derivatives, formamidine sulfonic acid, silane compounds) and a metal sensitization method using a metallic compound (e.g., gold complex salts and complex salts of Group VIII metals such as Pt, Ir, Pd, Rh and Fe). These sensitization methods may be used either alone or in a combination of two or more.

Among these chemical sensitization methods, the sulfur sensitization method and/or the gold sensitization method are/is preferred and the sulfur sensitization method alone is particularly preferred.

These sensitization methods are described in more detail in JP-A-62-215272 (page 12 the third column line 18 to the fourth column line 16) (the term "JP-A" as used herein means an "unexamined published Japanese patent application").

The silver chlorobromide emulsions of the present invention can be prepared according to the methods described in P. Glafkides, *Chemie et Physique Photographic* (Paul Montel, 1967); G. F. Duffin, *Photographic Emulsion Chemistry* (Focal Press, 1966); and V. L. Zelikan et al, *Making and Coating Photographic Emulsion* (Focal Press, 1966). Namely, any of the acid processes, the neutral processes and the ammonia processes can be used. In the stage of preparation, a soluble silver salt and a soluble halogen salt can be reacted in accordance with a single jet process, a double jet process or a combination thereof. A reverse mixing method in which grains are formed in the presence of excess silver ion can also be used. Further, a controlled double jet process can be used in which the pAg in a liquid phase where the silver halide grains are formed is kept constant. According to this method, there can be obtained a silver halide emulsion in which the crystal form is regular and the grain size is nearly uniform.

Generally, the silver halide emulsions of the present invention are spectrally sensitized.

Spectral sensitization is carried out for the purpose of imparting spectral sensitization in the desired wavelength of light to the emulsion of each layer of the photographic materials of the present invention. It is pre-

ferred that spectral sensitization is conducted by adding a dye which absorbs light in the wavelength corresponding to the desired spectral sensitivity of the invention, namely a spectral sensitizing dye. Examples of spectral sensitizing dyes which can be used are described in F. M. Harmer, *Heterocyclic Compounds-Cyanine Dyes and Related Compounds* (John Wiley & Sons, New York, London, 1964). Concrete examples thereof include compounds described in JP-62-215272 (pages 22-38).

Various compounds or precursors thereof may be added to the silver halide emulsions of the present invention for the purpose of preventing fogging from being caused during the preparation of the photographic materials, during the storage thereof or during processing, or for the purpose of stabilizing the photographic performance. These compounds are generally called photographic stabilizers. Preferred examples of these compounds are described in the aforesaid JP-A-62-215272 (pages 39-72).

The emulsions of the present invention may be any type of a surface latent image type emulsion wherein the latent image is predominantly formed on the surface of the grain, and the internal image type emulsion wherein the latent image is predominantly formed in the interior of the grain.

As described above, the photographic materials of the present invention are highly sensitive and have a low amount of fog. The characteristics of the present invention can be effectively exhibited when the sum total of the dry thickness (dried at 25° C., 55% RH for one week) of a hydrophilic coated material obtained by coating a support with the silver halide emulsion of the present invention is not more than 15  $\mu\text{m}$ , the wet thickness is in the range of 20 to 40  $\mu\text{m}$  and the 5-pyrazolone coupler having an elimination group represented by the general formula (I) is incorporated. It is known that it is advantageous in accelerating the development rate to have a film thickness during drying (dry thickness) which is small and to have a film thickness during wetting (wet thickness) which is large. However, when the emulsion containing the metal ion and the coupler of the present invention is used, a problem is caused wherein uneven development and stain are liable to result when the film thickness during wetting is too large. Therefore, the film thickness during wetting (wet thickness) must be kept 40  $\mu\text{m}$  or below. The term "film thickness during wetting" or "wet thickness" as used herein refers to thickness after the coated material is immersed in distilled water at 35° C. for 3 minutes.

5-pyrazolone couplers having an elimination group represented by general formula (I) will be illustrated below.

In the present invention, where the acyl group, the sulfonyl group, the sulfonamido, etc., are not specifically defined, they include aliphatic and aromatic groups thereof, and where the heterocyclic group is not specifically defined it preferably a 5- to 7-membered heterocyclic group containing at least one of S, O and N atoms as a hetero atom.

$L_1$  and  $L_2$  each represents a substituted or unsubstituted methylene or ethylene group. The groups which may be substituted thereon include halogen atoms (fluorine, chlorine, bromine, etc.), aliphatic groups (e.g., 1-22C straight chain or branched chain alkyl, aralkyl, alkenyl, alkynyl, cycloalkyl or cycloalkenyl), aryl groups (e.g., phenyl, naphthyl), heterocyclic groups (e.g., 2-furyl, 3-pyridyl), alkoxy groups (e.g., methoxy,

ethoxy, cyclohexyloxy), aryloxy groups (e.g., phenoxy, p-methoxyphenoxy, p-methylphenoxy), alkylamino groups (e.g., ethylamino, dimethylamino), alkoxy carbonyl groups (e.g., methoxycarbonyl, ethoxycarbonyl), carbamoyl groups (e.g., N,N-dimethylcarbamoyl), anilino groups (e.g., phenylamino, N-ethylanilino), sulfamoyl groups (e.g., N,N-diethylsulfamoyl), alkylsulfonyl groups (e.g., methylsulfonyl), arylsulfonyl groups (e.g., tolylsulfonyl), alkylthio groups (e.g., methylthio, octylthio), arylthio groups (e.g., phenylthio, 1-naphthylthio), acyl groups (e.g., acetyl, benzoyl), acylamino groups (e.g., acetamido, benzamido), imido groups (e.g., succinimide, phthalimide), ureido groups (e.g., phenylureido, N,N-dibutylureido), sulfamoylamino groups (e.g., N,N-dipropylsulfamoylamino), alkoxy carbonylamino groups (e.g., methoxycarbonylamino), sulfonamido groups (e.g., methanesulfonamide), a hydroxyl group and a cyano group, etc. Preferably,  $L_1$  and  $L_2$  are unsubstituted methylene and ethylene groups. 1 and m each represents 0 or 1 and are preferably 0.

$R_1$  represents a hydrogen atom, an alkyl group, an aryl group or a heterocyclic group. In more detail,  $R_1$  represents a hydrogen atom, an aliphatic group such as a 1-22C straight chain or branched chain alkyl group, alkenyl group or cycloalkyl group, an aryl group such as a phenyl or a naphthyl group or a heterocyclic group such as a 2-furyl, 2-thienyl, 2-pyrimidinyl or 4-pyridyl group. These may also have the substituent thereon that were defined for  $L_1$  and  $L_2$ . Preferably,  $R_1$  is a hydrogen atom or an alkyl group.

$R_2$  represents a group that is linked to A by a carbon, oxygen, nitrogen or sulfur atom. In more detail,  $R_2$  represents a group that is linked by a carbon atom such as an alkyl group, an aryl group, a heterocyclic group (linked by a carbon atom), an acyl group, an alkoxy carbonyl group or a carbamoyl group (linked by a carbon atom); a group that is linked by an oxygen atom such as an alkoxy group or an aryloxy group; a group that is linked by a nitrogen atom such as an alkylamino, anilino, acylamino, ureido, sulfamoylamino, alkoxy carbonylamino or sulfonamido group; or a group that is linked by a sulfur atom such as an alkylthio group or an arylthio group. Like  $R_1$ ,  $R_2$  may also have the substituent thereon that were defined for  $L_1$  and  $L_2$ . Preferably,  $R_2$  is an alkyl, aryl, alkylamino or anilino group.

A represents a carbon atom or a sulfur atom and is preferably a carbon atom.

n is 1 when A is a carbon atom and is 1 or 2 when A is a sulfur atom.

B represents a carbon, oxygen, nitrogen or sulfur atom and is preferably a carbon or nitrogen atom and still more preferably a carbon atom.

X represents a group of atoms necessary for forming a ring and is preferably a group that is necessary for forming a saturated or unsaturated 5, 6 or 7 membered ring and is constituted by atoms selected from among carbon, oxygen, nitrogen and sulfur atoms. More preferably, X is a group that is needed for forming an unsaturated 5 or 6 membered ring and is constituted by atoms selected from among carbon, oxygen and nitrogen atoms. These rings may also have a substituent thereon that were defined for  $L_1$  and  $L_2$  and other rings may be condensed onto the ring containing X.

$R_1$  and  $R_2$  may be bonded to one another and form a ring and may preferably form a 5- or 6-membered saturated or unsaturated ring. Such rings may also have the substituent thereon that was defined for  $L_1$  and  $L_2$ .

When B is a carbon atom or a nitrogen atom, B and R<sub>2</sub> may be bonded to one another to form a ring and they may suitably form a 5- or 6-membered saturated or unsaturated ring, a 5- or 6-membered saturated ring being preferred. Such rings may also have the substituent thereon that was defined for L<sub>1</sub> and L<sub>2</sub>.  
5

A first preferred pyrazolone coupler is represented by the following general formula:



wherein Y<sub>1</sub> in this general formula represents R<sub>a</sub> or Z<sub>1</sub>R<sub>b</sub>; R<sub>a</sub> represents a substituted or an unsubstituted aryl or a heterocyclic group or a substituent possessing a secondary or tertiary group represented by  
20



and i represents 0 or 1; Z<sub>1</sub> represents an oxygen atom, a sulfur atom or NRf; R<sub>b</sub> is a substituted or an unsubstituted alkyl, aryl or heterocyclic group; Rc and Rd each represents halogen atoms or groups selected from the groups consisting of R<sub>b</sub> and Z<sub>2</sub>Rg; Re is a hydrogen atom or a group as defined for Rc and Rd; Rf is a hydrogen atom or a group as defined for R<sub>b</sub>; Z<sub>2</sub> represents an oxygen atom or a sulfur atom or NRh; Rg is a group as defined for Rf; Rh is a group as defined for Rf; Rc may bond with Rd and/or Re to form one or two carbon rings or hetero rings and these may also possess substituents. R<sub>1</sub>, X and B signify the same groups, atomic groups and atoms as noted earlier; R<sub>3</sub> is an anilino, acylamino, ureido, carbamoyl, alkoxy, allyloxycarbonyl, alkoxy carbonyl or N-heterocyclic group and preferably these groups are groups containing oil-solubilizing groups. R<sub>4</sub> is a substituted or an unsubstituted aryl group and is preferably a substituted phenyl group, more preferably a 2,4,6-trichlorophenyl group.  
35  
40  
45

Preferred pyrazolone couplers of this general formula can be represented by the following general formula in which R<sub>1</sub>, R<sub>3</sub>, R<sub>4</sub>, Rc, Rd, Re, X and B signify the same atoms, atomic groups or groups as noted above and i is 0 or 1;  
50  
55



10  
15  
20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410  
8415  
8420  
8425  
8430  
8435  
8440  
8445  
8450  
8455  
8460  
8465  
8470  
8475  
8480  
8485  
8490  
8495  
8500  
8505  
8510  
8515  
8520  
8525  
8530  
8535  
8540  
8545  
8550  
8555  
8560  
8565  
85

wherein R<sub>1</sub>, R<sub>3</sub> and R<sub>4</sub> each signifies the same atoms and groups as noted above. R<sub>6</sub> and R<sub>7</sub> each represents alkyl or aryl groups and R<sub>8</sub> represents the substituents as defined for L<sub>1</sub> and L<sub>2</sub>. D represents a methylene group or an oxygen, nitrogen or sulfur atom and n represents an integer from 0 to 2 when it is a methylene group and is 1 in the other cases. p is an integer from 0 to 3.

The phrase "coupler moiety" discussed hereinbelow is the portion excluding the coupling elimination group. The term "coupler" refers to the entire body including both the coupler moiety and the coupling elimination group.

The coupling moiety reacts with an oxidized color development agent to form a dye and more specifically a magenta dye which is a pyrazolone coupler that is well-known and in common use in the photographic industry. Representative examples of suitable pyrazolone coupler moieties that may be cited include the substances disclosed in U.S. Pat. Nos. 4,413,054, 4,443,536, 4,522,915, 4,336,325, 4,199,361, 4,351,897, and 4,385,111, JP-A-60-170854, JP-A-60-194452 and JP-A-60-194451, U.S. Pat. Nos. 4,407,936, 3,419,391 and 3,311,476, UK Patent 1,357,372 and U.S. Pat. Nos. 2,908,573, 2,908,573, 3,062,653, 3,519,429, 3,152,896, 2,311,082, 2,343,703 and 2,369,489 and in the inventions cited in these patents. When the coupling elimination groups are substituted on the pyrazolone coupler moieties of these patents, it is possible to effect replacement with the coupling elimination groups represented by general formula (I) of the present invention. The pyrazolone couplers of the invention can also be used together with other pyrazolone couplers disclosed in the patents noted above.

Examples of preferred coupler moieties are represented in the following general formula:



wherein Q represents a coupling elimination group of the invention; R<sub>9</sub> is an anilino, acylamino, ureido, carbamoyl, alkoxy, aryloxycarbonyl, alkoxy carbonyl or N-heterocyclic group; R<sub>10</sub> is a substituted or an unsubstituted aryl group and is preferably a phenyl group with at least one substituent selected from among halogen atoms and alkyl, alkoxy, alkoxy carbonyl, acylamino, sulfamido, sulfonamido and cyano groups. The carbon atoms and the nitrogen atoms of these substituents may be unsubstituted or substituted by groups which do not reduce the coupler's effects. R<sub>9</sub> is preferably an anilino group and is more preferably an anilino group represented by the following general formula:



wherein R<sub>11</sub> is a 1-30C alkoxy group, aryloxy group or halogen atom (preferably a chlorine atom); R<sub>12</sub> and R<sub>13</sub> are respectively hydrogen atoms, halogen atoms (e.g.,

chlorine, bromine, fluorine), alkyl groups (e.g., 1-30C alkyl groups), alkoxy groups (e.g., 1-30C alkoxy groups) or acylamino, sulfonamido, sulfamoyl, sulfamido, carbamoyl, diacylamino, aryloxycarbonyl, alkoxy carbonyl, alkoxy sulfonyl, aryloxysulfonyl, alkanesulfonyl, arylsulfonyl, alkylthio, arylthio, alkoxy carbonylamino, alkylureido, acyl, nitro or carboxyl groups. For example, R<sub>12</sub> and R<sub>13</sub> may each be a hydrogen atom or a ballast group.

R<sub>10</sub> is preferably a substituted phenyl group. The substituents thereof include halogen atoms (e.g., chlorine, bromine, fluorine), 1-22C alkyl groups (e.g., methyl, ethyl, propyl, t-butyl, tetradearyl), 1-22C alkoxy groups (e.g., methoxy, ethoxy, dodecyloxy), 1-23C alkoxy carbonyl groups (e.g., methoxycarbonyl, ethoxycarbonyl, tetradecyloxycarbonyl), acylamino groups (e.g.,  $\alpha$ -(3-pentadecylphenoxy)-butylamide) and/or amino groups. More preferably, R<sub>10</sub> is a 2,4,6-trichlorophenyl group.

More specifically, R<sub>12</sub> and R<sub>13</sub> include hydrogen atoms, halogen atoms (e.g., chlorine, bromine, fluorine), 1-30C straight chain or branched chain alkyl groups (e.g., methyl, trifluoromethyl, ethyl, t-butyl, tetradearyl), 1-30C alkoxy groups (e.g., methoxy, ethoxy, 2-ethylhexyloxy, tetradecyloxy), acylamino groups (e.g., acetamido, pentylphenoxyacetamide,  $\alpha$ -(2,4-di-t-pentylphenoxy)butylamido,  $\alpha$ -(4-hydroxy-3-t-butylphenoxy)tetradecaneamido, 2-oxopyrrolidin-1-yl, 2-oxy-5-tetradecylpyrrolin-1-yl, N-methyltetradecaneamido, t-butylcarbonamido), sulfonamido groups (e.g., methanesulfonamido, benzenesulfonamido, p-toluenesulfonamido, p-dodecylbenzenesulfonamido, N-methyltetradecylsulfonamido, hexadecanesulfonamido), sulfamoyl groups (e.g., N-methylsulfamoyl, N-hexadecylsulfamoyl, N,N-dimethylsulfamoyl, N-(3-(dodecyloxy)propyl)sulfamoyl, N-(4-(2,4-di-t-pentylphenoxy)butyl)sulfamoyl, N-methyl-N-tetradecylsulfamoyl, N-dodecylsulfamoyl), sulfamido groups (e.g., N-methylsulfamido, N-octadecylsulfamido), carbamoyl groups (e.g., N-methylcarbamoyl, N-octadecylcarbamoyl, N-(4-(2,4-di-t-pentylphenoxy)butyl)carbamoyl, N-methyl-N-tetradecylcarbamoyl, N,N-diethylcarbamoyl), diacylamino groups (e.g., N-succinimido, N-phthalimido, 2,5-dioxo-1-oxazolidinyl, 3-dodecyl-2,5-dioxo-1-imidazolyl, N-acetyl-N-dodecylamino), aryloxycarbonyl groups (e.g., phenoxycarbonyl, p-dodecyloxyphenoxy carbonyl), 2-30C alkoxy carbonyl groups (e.g., methoxycarbonyl, tetradecyloxycarbonyl, ethoxycarbonyl, benzoyloxycarbonyl, dodecyloxycarbonyl), 1-30C alkoxy sulfonyl groups (e.g., methoxysulfonyl, octyloxysulfonyl, tetradecyloxysulfonyl, 2-ethylhexyloxysulfonyl), aryloxysulfonyl groups (e.g., phenoxy sulfonyl, 2,4-di-t-pentylphenoxy sulfonyl), 1-30C alkanesulfonyl groups (e.g., methanesulfonyl, octanesulfonyl, 2-ethylhexanesulfonyl, hexadecanesulfonyl), arylsulfonyl groups (e.g., benzenesulfonyl, 4-nonylbenzenesulfonyl, p-toluenesulfonyl), 1-22C alkylthio groups (e.g., ethylthio, octylthio, benzylthio, tetradecylthio, 2-(2,4-di-t-pentylphenoxy)ethylthio), arylthio groups (e.g., phenylthio, p-tolylthio), alkoxy carbonylamino groups (e.g., ethoxycarbonylamino, benzoyloxycarbonylamino, hexadecyloxycarbonylamino), alkylureido groups (e.g.,

65 N-methylureido, N,N-dimethylureido, N-methyl-N-dodecylureido, N-hexadecylureido, N,N-diocadecylureido, N,N-dioctyl-N'-ethylureido), acyl groups (e.g., acetyl, benzoyl, octadecanoyl, p-

35 40 45 50 55 60 65

35 40 45 50 55 60 65

35 40 45 50 55 60 65

dodecaneamidobenzoyl, cyclohexanecarbonyl), nitro groups, cyano groups and carboxyl groups.

The alkoxy and aryloxy groups of  $R_{11}$  further include the case where the alkoxy groups are methoxy, ethoxy, propoxy, butoxy, 2-methoxyethoxy, sec-butoxy, hex-5 yloxy, 2-ethylhexyloxy, 2-(2,4-di-t-pentylphenoxy)ethoxy and 2-dodecyloxyethoxy groups and the aryloxy groups are phenoxy,  $\alpha$  and  $\beta$ -naphthoxy and 4-tolyloxy groups.

A monomer containing a pyrazolone coupler with 10 the elimination group represented by general formula (I) may serve to form a copolymer with a non-color-forming ethylenic monomer which does not couple with the oxidation products of primary aromatic amine developing agents.

Representative examples of non-color-forming ethylenic monomers which do not couple with the oxidation products of primary aromatic amine developing agents include acrylic acid,  $\alpha$ -chloroacrylic acid,  $\alpha$ -alkylacrylic acid (e.g., methacrylic acid) and esters or amides 20 derived from these acrylic acids (e.g., acrylamide, n-butylacrylamide, t-butylacrylamide, diacetoneacrylamide, methacrylamide, methyl acrylate, ethyl acrylate, n-propyl acrylate, n-butyl acrylate, t-butyl acrylate, 25 isobutyl acrylate, 2-ethylhexyl acrylate, n-octyl acrylate, lauryl acrylate, methyl methacrylate, ethyl methacrylate, n-butyl methacrylate, and  $\beta$ -hydroxy methacrylate), methylene bisacrylamide, vinyl esters (e.g., vinyl acetate, vinyl propionate and vinyl laurate), acrylonitrile, methacrylonitrile, aromatic vinyl compounds 30 (e.g., styrene and derivatives thereof, vinyltoluene, divinylbenzene, vinylacetophenone and sulfostyrene), itaconic acid, citraconic acid, crotonic acid, vinylidene chloride, vinyl alkyl ethers (e.g., vinyl ethyl ether), maleic acid, maleic anhydride, maleic acid esters, N-35 vinyl-2-pyrrolidone, N-vinylpyridine and 2 or 4-vinylpyridine, etc. Two or more non-coloring unsaturated 40 ethylenic monomers may be used together. For example, one can have n-butyl acrylate and methylacrylate, styrene and methacrylic acid, methacrylic acid and acrylamide or methyl acrylate and diacetone acrylamide, etc.

As is well-known in the field of polymer color couplers, it is possible to select noncoloring unsaturated 45 ethylenic monomers for copolymerization with solid, water-soluble monomers in such a manner as to have good effects on the physical and/or chemical properties of the copolymer that is formed, e.g., solubility, compatibility with photographic colloid composition binders, for example, gelatin and the pliability and thermal 50 stability, etc. of the copolymer.

Polymer couplers used in the invention may be water 55 soluble or water-insoluble, but within the various substances polymer coupler latexes are particularly preferred.

Below, specific examples of coupling elimination groups Q that are represented by general formula (I) are given, although there is no limitation to these examples.

-continued

Q-2)



Q-3)



Q-4)



Q-5)



Q-6)



Q-7)



Q-8)



Q-9)



**15**  
-continued



5,250,407

**16**

-continued



**17**

-continued



**5,250,407**

**18**

-continued



**19**

-continued



**5,250,407**

**20**

-continued

Q-44)

5



Q-45)

10



Q-46)

15



Q-47)

20



Q-48)

25



Q-49)

30



Q-50)

35



Q-51)

40



Q-52)

45



Q-53)

50



Q-54)

55



Q-55)

60



Q-56)

65



Q-57)



Q-60)

Specific examples of the couplers of the present invention will now be given, although the invention is not limited to these representative examples.

(M-1)



(M-2)



(M-3)



-continued

(M-4)



(M-5)



(M-6)



(M-7)



-continued



(M-8)



(M-9)



(M-10)



(M-11)



-continued

(M-12)



(M-13)



(M-14)



(M-15)

-continued



(M-17)



(M-18)



(M-19)



-continued

(M-20)



(M-21)



(M-22)



(M-23)



-continued



-continued



(M-28)



(M-29)



(M-30)



(M-31)

-continued

(M-32)



(M-33)



(M-34)



(M-35)



-continued

(M-36)



(M-37)



(M-38)



(M-39)



-continued

(M-40)



(M-41)



(M-42)



(M-43)



-continued

(M-44)



(M-45)



(M-46)



(M-47)



45

5,250,407

46

-continued



(M-48)



(M-49)



(M-50)



(M-51)

-continued

(M-52)



(M-53)



(M-54)



-continued



(M-55)



(M-56)



(M-57)



(M-58)

-continued



(M-59)



-continued

(M-63)



(M-64)



(M-65)



(M-66)



The magenta couplers of the present invention are used in an amount of  $1 \times 10^{-3}$  mol to 1 mol, preferably

The magenta couplers of the present invention may be arbitrarily added to the silver halide emulsion layers. However, it is preferred that the magenta couplers of the present invention are added to the green-sensitive silver halide emulsion layer. The amount of silver used in this green-sensitive silver halide emulsion layer is preferably 0.1 to 0.3 g/m<sup>2</sup>.

The magenta couplers of the present invention can be synthesized according to the method described in WO88/04795.

Normally, yellow couplers, magenta couplers and cyan couplers which couple with the oxides of aromatic amine developing agents to produce the respective colors yellow, magenta and cyan are used in a color photographic material.

Acylacetamide derivatives such as benzoylacetoanilide and pivaloylacetoaniline are preferred as yellow couplers for use in the invention.

Of these substances, substances represented by the following general formulas (Y-1) and (Y-2) are suitable as yellow couplers:



wherein X represents an hydrogen atom or a coupling elimination group; R<sub>21</sub> represents a 8-32C diffusion-resistant group; R<sub>22</sub> represents a hydrogen atom, 1 or more halogen atoms, or a lower alkyl (preferably having lower alkoxy (preferably having 1-4C) or 8-32C diffusion-resistant group; R<sub>23</sub> represents a hydrogen atom or a substitution group. When there are two or more R<sub>23</sub>s, they may be the same or different. R<sub>24</sub> repre-

sents a halogen atom, an alkoxy group a trifluoromethyl group or an aryl group. R<sub>25</sub> represents a hydrogen atom, a halogen atom or an alkoxy group. A represents —NHCOR<sub>26</sub>, —NHSO<sub>2</sub>R<sub>26</sub>, —SO<sub>2</sub>NHR<sub>26</sub>,



10 wherein R<sub>26</sub> and R<sub>27</sub> each represents an alkyl group, an aryl group or an acyl group.

Details of pivaloylacetoanilide yellow couplers are disclosed in the Specifications of U.S. Pat. No. 4,622,287, column 3 line 15 to column 8 line 39, and U.S.

15 Pat. No. 4,623,616, column 14 line 50 to column 19 line 41.

Details of benzoylacetoanilide yellow couplers are disclosed in U.S. Pat. Nos. 3,408,194, 3,933,501, 4,046,575, 4,133,958 and 4,401,752, etc.

The compounds (Y-1) to (Y-39) disclosed in column 37 to column 54 of the abovenoted U.S. Pat. No. 4,622,287 may be cited as specific examples of pivaloylacetoanilide yellow couplers, (Y-1), (Y-4), (Y-6), (Y-7), (Y-15), (Y-21), (Y-22), (Y-23), (Y-26), (Y-35), (Y-36), (Y-37), (Y-38) and (Y-39), etc. with these being preferred.

One may also cite the examples of compounds (Y-1) to (Y-33) on column 19 to column 24 of the abovenoted U.S. Pat. No. 4,623,616, (Y-2), (Y-7), (Y-8), (Y-12), 30 (Y-20), (Y-21), (Y-23) and (Y-29), etc. with these being suitable.

Apart from these examples, one may also cite as suitable substances the typical specific example (34) disclosed in column 6 of the Specification of U.S. Pat. Nos.

35 3,408,194, the compounds (16) and (19) disclosed in column 8 of the Specification of U.S. Pat. No. 3,933,501, compound (9) disclosed in columns 7 to 8 of the Specification of U.S. Pat. No. 4,046,575, compound (1) disclosed in columns 5 and 6 of the Specification of U.S.

40 Pat. No. 4,133,958, compound 1 disclosed in column 5 of the Specification of U.S. Pat. No. 4,401,752 and the compounds a) to h) indicated below:



| Compound | A | X |
|----------|---|---|
| a        |   |   |

-continued



| Compound | A | X |
|----------|---|---|
| b        |   |   |
| c        |   |   |
| d        |   |   |
| e        |   |   |
| f        |   |   |
| g        |   |   |
| h        |   |   |

Among these couplers, the couplers in which the elimination atoms are nitrogen atoms are particularly preferred.

Other magenta couplers that are employable together with the pyrazolone magenta couplers that are used in the invention include, for example, oil-protected type 65 couplers, indazolone couplers, cyanoacetyl couplers and preferably pyrazoloazole couplers, such as pyrazolotriazole or 5-pyrazolone couplers. Within the

5-pyrazolone type couplers, couplers in which the 3 position is substituted by an arylamino or an acylamino group are preferable from the point of view of the hue of the dye and the density of the color produced. Typical examples of such couplers are disclosed in U.S. Pat. Nos. 2,311,082, 2,343,703, 2,600,788, 2,908,573, 3,062,653, 3,152,896 and 3,936,015, etc. The nitrogen

atom elimination groups disclosed in U.S. Pat. No. 4,310,619 and the arylthio elimination groups disclosed in U.S. Pat. No. 4,351,897 are preferred as elimination groups for the 2-equivalent 5-pyrazolone couplers. 5 Good color density is also achievable with the 5-pyrazolone couplers possessing the ballast groups disclosed in European Patent 73,636.

The pyrazolobenzimidazoles disclosed in U.S. Pat. No. 2,369,879 and, preferably, the pyrazolo(5,1-c)-(1,2,4)triazoles disclosed in U.S. Pat. No. 3,725,067, the pyrazolotetrazoles disclosed in *Research Disclosure* 24220 (June 1984) and the pyrazolopyrazoles disclosed in *Research Disclosure* 24230 (June 1984) may be cited as 15 pyrazoloazole couplers. All of the above couplers may be polymer couplers.

Specific examples of the couplers are represented by 20 the following general formulas (M-1), (M-2) and (M-3):



wherein R<sub>31</sub> represents a 8-32C diffusion-resistant group and R<sub>32</sub> represents a phenyl or a substituted phenyl group; R<sub>33</sub> represents a hydrogen atom or a substituent; Z represents a group of nonmetal atoms necessary for forming a 5-membered azole ring containing 2 to 4 nitrogen atoms and substituents (including condensed rings) may be substituted to this azole ring.

X<sub>2</sub> represents a hydrogen atom or a group that is capable of eliminating. Details of substituents of R<sub>33</sub> and the azole ring substitution groups are disclosed in, e.g., column 2 line 41 to column 8 line 27 of the Specification of U.S. Pat. No. 4,540,654.

Within the pyrazoloazole couplers, the imidazo(1,2-b)pyrazoles disclosed in U.S. Pat. No. 4,500,630 are preferred and the pyrazolo(1,5-b)(1,2,4)triazoles disclosed in U.S. Pat. No. 4,540,654 are particularly preferred since there is little yellow side absorption and good light fastness of the coupler dye.

Apart from these couplers, pyrazolotriazole couplers with branched alkyl groups directly connected to the 2, 3 or 6 positions of the pyrazolotriazole ring as disclosed in JP-A-61-65245, pyrazoloazole couplers containing sulfonamido groups in their molecules as disclosed in JP-A-61-65246, pyrazoloazole couplers with alkoxy-phenylsulfonamido ballast groups as disclosed in JP-A-61-147254 and pyrazolotriazole couplers with an alkoxy group or aryloxy group in the 6 position as disclosed in European Patent (Laid-open) 226,849 are suitable for use.

Specific examples of these couplers are as follows.

| Compound | R <sub>33</sub> | R <sub>34</sub> | R <sub>14</sub> | X <sub>2</sub> |
|----------|-----------------|-----------------|-----------------|----------------|
| M'-1     |                 |                 |                 | Cl             |
| M'-2     |                 |                 |                 | Cl             |
| M'-3     |                 |                 |                 |                |
| M'-4     |                 |                 |                 |                |

-continued

| Compound | R <sub>33</sub>   | R <sub>34</sub>                                               | R <sub>35</sub>                 | X <sub>2</sub> |
|----------|-------------------|---------------------------------------------------------------|---------------------------------|----------------|
| M'-5     | CH <sub>3</sub> — | OC <sub>2</sub> H <sub>4</sub> OC <sub>2</sub> H <sub>5</sub> | OC <sub>8</sub> H <sub>17</sub> | Cl             |
|          |                   |                                                               |                                 |                |
| M'-6     | CH <sub>3</sub> — |                                                               |                                 | Cl             |
|          |                   |                                                               |                                 |                |
| M'-7     |                   |                                                               |                                 |                |
|          |                   |                                                               |                                 |                |
| M'-8     |                   |                                                               |                                 | as above       |
| M'-9     |                   |                                                               |                                 | as above       |
|          |                   |                                                               |                                 |                |
|          |                   |                                                               |                                 |                |

-continued

| Compound | R <sub>33</sub> | R <sub>34</sub> | X <sub>2</sub> |
|----------|-----------------|-----------------|----------------|
| M'-10    |                 |                 | Cl             |
| M'-11    |                 |                 | Cl             |
| M'-12    |                 |                 | Cl             |
| M'-13    |                 |                 | Cl             |
| M'-14    |                 |                 | Cl             |

-continued

| Compound | R <sub>33</sub> | R <sub>34</sub> | X <sub>2</sub>                     |
|----------|-----------------|-----------------|------------------------------------|
| M'-15    |                 |                 | Cl                                 |
| M'-16    |                 |                 | C <sub>8</sub> H <sub>17</sub> (t) |

(The monomer ratio is shown by weight.)

The most representative cyan couplers are phenolic cyan couplers and naphtholic cyan couplers.

Phenolic cyan couplers comprise the couplers (including the polymer couplers) disclosed in U.S. Pat. Nos. 2,369,929, 4,518,687, 4,511,647 and 3,772,002 which have an acylamino group in the 2 position and an alkyl group in the 5 position of a phenol nucleus. Representative specific examples of these couplers include the coupler of Example 2 disclosed in Canadian Patent 625,822, Compound (1) disclosed in U.S. Pat. No. 3,772,002, Compounds (I-4) and (I-5) disclosed in U.S. Pat. No. 4,564,590, Compounds (1), (2), (3) and (24) disclosed in JP-A-61-39045 and Compound (C-2) disclosed in JP-A-62-70846.

Phenolic cyan couplers also include the 2,5-diacylaminophenolic couplers disclosed in U.S. Pat. Nos. 2,772,162, 2,895,826, 4,334,011 and 4,500,653 and JP-A-59-164555 and representative specific examples of these couplers include Compound (V) disclosed in U.S. Pat. No. 2,895,826, Compound (17) disclosed in U.S. Pat. No. 4,557,999, Compounds (2) and (12) disclosed in U.S. Pat. No. 4,565,777, Compound (4) disclosed in U.S. Pat. No. 4,124,396 and Compound (I-19) disclosed in U.S. Pat. No. 4,613,564.

5 Additional examples of phenolic cyan couplers include those couplers disclosed in U.S. Pat. Nos. 4,327,173, 4,564,586 and 4,430,423, JP-A-62-257158 and JP-A-62-257158 in which the nitrogen-containing heterocyclic rings are fused to phenol nuclei. Representative specific examples of these couplers that may be cited include Couplers (1) and (3) disclosed in U.S. Pat. No. 4,327,173, Compounds (3) and (16) disclosed in U.S. Pat. No. 4,564,586, Compounds (1) and (3) disclosed in U.S. Pat. No. 4,430,423 and the following compounds:



25



-continued



Apart from the abovenoted types of cyan couplers, one may also use, for instance, the diphenylimidazole cyan couplers disclosed in Laid-open European Patent EP0,249,453A2.





Phenolic cyan couplers further include the ureido 23  
couplers disclosed in U.S. Pat. Nos. 4,333,999,  
4,451,559, 4,444,872, 4,427,767 and 4,579,813 and European Patent (EP) 067,689B1. Representative specific examples of these couplers that may be cited include Coupler (7) disclosed in U.S. Pat. No. 4,333,999, Coupler (1) disclosed in U.S. Pat. No. 4,451,559, Coupler (14) disclosed in U.S. Pat. No. 4,444,872, Coupler (3) disclosed in U.S. Pat. No. 4,427,767, Couplers (6) and (24) disclosed in U.S. Pat. No. 4,609,619, Couplers (1) and (11) disclosed in U.S. Pat. No. 4,579,813, Couplers (45) and (50) disclosed in European patent (EP) 067,689B1 and Coupler (3) disclosed in JP-A-61-42658. 30 33

Naphtholic cyan couplers include couplers which have an N-alkyl-N-arylcarbamoyl group in the 2 position of their naphthol ring (as in, e.g., U.S. Pat. No. 2,313,586), couplers with an alkylcarbamoyl group in the 2 position (as in, e.g., U.S. Pat. No. 2,474,293 and 4,282,312), couplers with an arylcarbamoyl group in the 2 position (as in, e.g., JP-B-50-14523 (the term "JP-B" as used herein means an "examined Japanese patent publication"), couplers with a carbonamido or sulfonamido group in the 5 position (as in, e.g., JP-A-60-237448, JP-A-61-145557 and JP-A-61-153640), couplers with aryloxy elimination groups (as in, e.g., U.S. Pat. No. 3,476,563), couplers with substituted alkoxy elimination groups (as in, e.g., U.S. Pat. No. 4,296,199) and couplers with glycolic acid elimination groups (as in, e.g., JP-B-60-39217).

These couplers can be included in a dispersed emulsion layer in the presence of at least one high boiling point organic solvent. Preferably, high boiling point organic solvents represented by the following formulas (A) to (D) are used:



### Formula (A)



### Formula (B)

|    |                                                                                                                |             |
|----|----------------------------------------------------------------------------------------------------------------|-------------|
| 25 | $  \begin{array}{c}  \text{-continued} \\  \text{W}_2 \\  \text{W}_1-\text{CON} \\  \text{W}_3  \end{array}  $ | Formula (C) |
|    | $  \text{W}_1-\text{O}-\text{W}_2  $                                                                           | Formula (D) |

In formulas (A) to (D),  $W_1$ ,  $W_2$  and  $W_3$  each represent substituted or unsubstituted alkyl groups, cycloalkyl groups, alkenyl groups, aryl groups or heterocyclic groups,  $W_4$  represents  $W_1$ ,  $OW_1$  or  $S\text{-}W_1$  and  $n$  is an integer in the range of 1 to 5. When  $n$  is 2 or more, the  $W_4$ 's may be the same or different and  $W_1$  and  $W_2$  in general formula (E) may form condensed rings.

general formula (E) may form condensed rings. Details of these high boiling point organic solvents are disclosed on page 137, lower right-hand column to 40 page 144, upper right-hand column of the Specification of IP-A-62-215272

51-A-62-215272  
The above couplers can also be impregnated in a  
loadable latex polymer (as in, e.g., U.S. Pat. No.  
4,203,716) in the presence or the absence of a high-boil-  
45 ing point organic solvent or they may be dissolved in a  
polymer that is insoluble in water but soluble in an  
organic solvent and emulsified and dispersed in a hydro-  
philic colloid.

Preferably, use is made of the homopolymers or co-polymers disclosed on page 12 to page 30 of the Specification of Laid-open International Patent WO88/00723, and from the point of view of characteristics such as the stabilization of color images, use of acrylamide polymers is particularly preferred.

55 Antifoggants in the form of hydroquinone derivatives, aminophenol derivatives, gallic acid derivatives or ascorbic acid derivatives, etc. may be included in the photosensitive material used in the invention.

A variety of color fading preventives may be used in the photographic material of the invention. Representative examples of organic color fading preventives for cyan, magenta and/or yellow images include hydroquinones, 6-hydroxycromans, 5-hydroxycoumarans, spirocromans, hindered phenols, mainly p-alkoxyphenols and bisphenols, gallic acid derivatives, methylenedioxybenzenes, aminophenols, hindered amines and ether or ester derivatives in which the phenolic hydroxyl groups of these various compounds are sily-

lated or alkylated. Metal complexes, etc. such as typified by (bis-salicylaldoximato) nickel complexes and (bis-N,N-dialkyldithiocarbamato) nickel complexes may also be used.

Specific examples of organic color fading preventives are disclosed in the Specifications of the following patents. Hydroquinones are disclosed in, e.g., U.S. Pat. Nos. 2,360,290, 2,418,613, 2,700,453, 2,701,197, 2,728,659, 2,732,300, 2,735,765, 3,982,944 and 4,430,425, UK Patent 1,363,921 and U.S. Pat. Nos. 2,710,801 and 10 2,816,028; 6-hydrocromans, 5-hydroxycoumarans and spirocromans in e.g., U.S. Pat. Nos. 3,432,300, 3,573,050, 3,574,627, 3,698,909 and 3,764,337 and JP-A-52-152225; spiroindanes in U.S. Pat. No. 4,360,589; p-alkoxyphenols in, e.g., U.S. Pat. No. 2,735,765, UK Patent 2,066,975, JP-A-59-10539 and JP-B-57-19765; hindered phenols in, e.g., U.S. Pat. No. 3,700,455, JP-A-15 52-72224, U.S. Pat. No. 4,228,235 and JP-B-52-6623; gallic acid derivatives, methylenedioxybenzenes and aminophenols in patents such as U.S. Pat. Nos. 3,457,079 and 4,332,886 and JP-B-56-21144; hindered amines in, e.g., U.S. Pat. Nos. 3,336,135 and 4,268,593, UK Patents 1,326,889, 1,354,313 and 1,410,846, JP-B-51 20 1420, JP-A-58-114036, JP-A-59-53846 and JP-A-59-78344; phenolic hydroxyl group ether and ester derivatives in, e.g., U.S. Pat. Nos. 4,155,765, 4,174,220, 4,254,216 and 4,264,720, JP-A-54-145530, JP-A-55-6321, JP-A-58-105147 and JP-A-59-10539, JP-B-57-35 37856, U.S. Pat. No. 4,279,990 and JP-B-53-3263; and, metal complexes in, e.g., U.S. Pat. Nos. 4,050,938 and 4,241,155 and UK Patent 2,027,731(A). The objects can be achieved by the addition to a photosensitive layer after co-emulsification of these various compounds with 40 couplers in amounts that are normally 5 to 100 wt % relative to the color couplers to which they correspond. Deterioration of cyan dye images due to heat and especially due to light can be more effectively prevented by the introduction of an ultraviolet ray absorption agent into the adjacent layers on both sides of the cyan coloring layer.

Particularly preferred color fading preventive agents among the abovenoted color fading preventives include spiroindanes and hindered amines.

Preferably in the invention, the compounds noted below are used together with the abovenoted couplers, especially with the pyrazolozazole couplers.

The use, alone or simultaneously, of compound (F) which bonds chemically with aromatic amine developing agents remaining after color development processing to form a compound that is chemically inert and essentially colorless and/or a compound (G) which bonds chemically with the oxides of the aromatic amine developing agent remaining after color development processing to form a chemically inert and essentially colorless compound is desirable from the point of view of preventing the occurrence of stains and other side effects due, for example, to a reaction between couplers and the residual developing agents or oxides thereof in the film during post-processing storage.

Preferred examples of compound (F) are compounds whose rate constant  $k_2$  of the secondary reaction with p-anisidine (in trioctyl phosphate at 80° C.) is in the range of  $1.0 \text{ l/mol}\cdot\text{sec} - 1 \times 10^{-5} \text{ l/mol}\cdot\text{sec}$ .

If  $k_2$  is above this range, the compound itself becomes unstable and may decompose through reaction with 65 gelatin and water. On the other hand, if  $k_2$  is below the above-mentioned range, the reaction with the residual aromatic amine developing agents is slow. Conse-

quently, there may be failure to achieve the object of the invention which is to prevent side effects from such residual aromatic amine developing agents.

Preferred forms of compound (F) can be represented by the following general formulas (FI) and (FII):



wherein  $R_1$  and  $R_2$  are each aliphatic, aromatic or heterocyclic groups;  $X$  represents a group which is eliminated by the reaction with an aromatic amine developing agent;  $A$  represents a group which forms a chemical bond by the reaction with the aromatic amine developing agent;  $n$  is 1 or 0.  $B$  is a hydrogen atom or an aliphatic, aromatic, heterocyclic, acyl or sulfonyl group;  $Y$  represents a group which accelerates the addition of the aromatic amine developing agent to the compound of general formula (FII);  $R_1$  and  $X$  may bond together and  $Y$  may bond with  $R_2$  or  $B$  to form ring structures.

Typical modes of chemical bonding with residual aromatic amine developing agents are bonding through a substitution reaction and bonding through an addition reaction.

Specific examples of compounds represented by general formulas (FI) and (FII) are given in JP-A-63-158545, JP-A-62-283338, JP-A-62-158342, and Japanese Patent Application 63-184349.

Details concerning combinations of the above-noted compound (G) and Compound (F) are given in Japanese Patent Application 63-18439.

Among the types of compound (G) which are chemically bonded to the oxidants of aromatic amine developing agents remaining after color development to form a colorless compound which is chemically inert, compounds represented by the following general formula (GI) are more preferred:



wherein  $R$  is an aliphatic group, an aromatic group or a heterocyclic group; and  $Z$  is a nucleophilic group or a group which releases a nucleophilic group in the photographic material. Among the compounds having the formula (GI), there are preferred compounds where  $Z$  is a group having a Rearson's nucleophilic  $^n\text{CH}_3$  I value [R. G. Rearson, et al., *J. Am. Chem. Soc.*, 90, 319 (1968)] of 5 or greater or a group derived therefrom.

Examples of the compounds having the formula (GI) are described in European Patent Laid-open No. 255722, JP-A-62-143048, JP-A-62-229145 and Japanese Patent Application Nos. 63-18439, 63-136724, 62-214681 and 62-158342.

Combinations of compounds (D) with compounds (F) are described in more detail in Japanese Patent Application No. 63-18439.

Preferably, amine compounds are used to prevent stain from being formed by colored dye formed by the reaction of couplers with color developing agents remaining during storage after processing or oxidants thereof, or to prevent other side effects from occurring. Among the amine compounds, compounds represented by the following general formula (FG) are preferred:



(FG)

In the formula (FG),  $\text{R}_{00}$  represents a hydrogen atom, a hydroxyl group, an alkoxy group, an acyloxy group, a sulfonyloxy group, a substituted or an unsubstituted amino group, an alkyl group, an aryloxy group, a heterocyclic oxy group, an aliphatic group, an aromatic group or a heterocyclic group;  $\text{R}_{01}$  represents a hydrogen atom, an aliphatic group, an aromatic group or a heterocyclic group; and  $\text{R}_{02}$  represents an aliphatic group, an aromatic group or a heterocyclic group. At least two of  $\text{R}_{00}$ ,  $\text{R}_{01}$  and  $\text{R}_{02}$  may be combined together to form a monocyclic or a polycyclic heterocyclic ring.

Concrete examples of the compounds having the formula (FG) are described in U.S. Pat. Nos. 4,483,918, 4,555,479 and 4,585,728, JP-A-58-102231 and JP-A-59-229557.

The hydrophilic colloid layers of the photographic materials of the present invention may contain ultraviolet light absorbers. Examples of the ultraviolet light absorbers include aryl group-substituted benzotriazole compounds (described in U.S. Pat. No. 3,533,794); 4-thiazolidone compounds (described in U.S. Pat. Nos. 3,314,794 and 3,352,681); benzophenone compounds (described in JP-A-46-2784); cinnamic ester compounds (described in U.S. Pat. Nos. 3,705,805 and 3,707,375); 25 butadiene compounds (described in U.S. Pat. No. 4,045,229); and benzococcidol compounds (described in U.S. Pat. No. 3,700,455). If desired, ultraviolet light absorbing couplers (e.g.,  $\alpha$ -naphthol cyan color-forming couplers) and ultraviolet light absorbing polymers 30 may be used. These ultraviolet light absorbers may be incorporated into specific layers.

Hydrophilic colloid layers in the photosensitive material produced by the invention may contain water soluble dyes as filter dyes or for the purpose of blocking 40 irradiation or for a variety of other purposes. Examples of such dyes include oxonol dyes, hemioxonol dyes, styryl dyes, merocyanine dyes, cyanine dyes and azo dyes. Among these dyes, oxonol, hemioxonol and merocyanine dyes are especially useful.

Furthermore, it is advantageous to use gelatin as a binder or as a protective colloid in the emulsion layers of the photographic material of the invention, although hydrophilic colloids other than gelatin may be used alone or together with gelatin.

The gelatin used in the invention may be either lime treated gelatin or gelatin that has been treated with acid. Details of gelatin manufacture are given in "The Macromolecular Chemistry of Gelatin" by Arthur Weiss (Academic Press, 1964).

Nitrocellulose film, or polyethylene terephthalate, or other such transparent film, or a reflecting support such as normally employed for photographic light-sensitive materials may be used as a support in the invention. From the point of view of the objects of the invention, 60 the use of a reflecting support is preferred.

What is meant by a "reflecting support" as used in the invention is a support which increases the reflectivity and thereby makes dye images formed in the silver halide emulsion layers sharper. These supports comprise elements in which a hydrophobic resin containing a dispersed reflecting substance such as titanium oxide, 65 zinc oxide, calcium carbonate or calcium sulfate, etc. is

coated on a support and elements in which a hydrophobic resin containing a dispersed reflecting substance is used as a support. There are, for example, supports making the joint use of a reflecting layer, and baryta paper, polyethylene coated paper or polypropylene synthetic paper, and transparent supports making the joint use of reflecting materials, e.g., glass plates, polyethylene terephthalate, cellulose triacetate, cellulose nitrate and similar polyester film, polyamide film, polycarbonate film, polystyrene film and vinyl chloride resin and one may select different supports in accordance with the intended use.

Reflecting materials are suitable materials into which a white pigment has been thoroughly kneaded in the presence of a surfactant. Preferably, use is made of materials in which the surfaces of the pigment grains have been treated with a divalent- tetravalent alcohol.

With regard to the occupied area ratio (%) per unit area defined by the fine white pigment grains, the most representative way of determining this is to divide the area that is under observation into the continuous unit areas of  $6 \mu\text{m} \times 6 \mu\text{m}$  and measure the ratio (%) ( $R_1$ ) of the projected area of the fine grains in these unit areas. The coefficient of variation of the occupied area ratio (%) can be determined by  $s/\bar{R}$  which is the ratio of  $R_1$ 's standard deviation  $s$  to the average value ( $\bar{R}$ ) of  $R_1$ . The number (n) of unit areas preferably at least 6. The coefficient of variation  $s/\bar{R}$  can be determined as follows:

$$\sqrt{\frac{\sum_{i=1}^n (R_1 - \bar{R})^2}{n-1}} / \frac{\sum_{i=1}^n R_1}{n}$$

In the invention, the coefficient of variation of the fine pigment grains occupied area ratio (%) is preferably 0.15 or less, 0.12 or less being particularly preferred. If this value is 0.08 or less, the dispersion characteristics of the grains are considered to be essentially uniform.

Known primary aromatic amine color developing agents are included in the color developing solutions used in the invention. Preferred examples are p-phenylenediamine derivatives, representative examples of which will now be given although there is no limitation to these agents.

D-1: N,N-Diethyl-p-phenylenediamine D-2: 2-Amino-5-diethylaminotoluene

D-3: 2-Amino-5-(N-ethyl-N-laurylarnino)toluene

D-4: 4-(N-Ethyl-N-(8-hydroxyethyl)amino)aniline

D-5: 2-Methyl-4-(N-ethyl-N-(8-hydroxyethyl)amino)aniline

D-6: 4-Amino-3-methyl-N-ethyl-N-(8-(ethanesulfonamido)ethyl)-aniline

D-7: N-(2-Amino-5-diethylaminophenylethyl)methanesulfonamide

D-8: N,N-Dimethyl-p-phenylenediamine

D-9: 4-Amino-3-methyl-N-ethyl-N-methoxyethyl aniline

D-10: 4-Amino-3-methyl-N-ethyl-N-8-ethoxyethyl aniline

D-11: 4-Amino-3-methyl-N-ethyl-N-8-butoxyethyl aniline

A particularly preferred derivative among these p-phenylenediamine derivatives is compound (D-6), that is, 4-amino-3-methyl-N-ethyl-N-(8-(ethanesulfonamido)ethyl)-aniline.

These p-phenylenediamine derivatives may also be in the form of salts such as sulfates, hydrochlorides, sulfites or p-toluenesulfonates, etc. The amount of the primary aromatic amine developing agent preferably used is such an amount as to give a concentration of about 0.1 g to about 20 g or more preferably, about 0.5 g to about 10 g per 1 liter of developing solution.

In the practice of the present invention, it is preferred to use developing solutions containing substantially no benzyl alcohol. The term "containing substantially no benzyl alcohol" as used herein means that the concentration of benzyl alcohol is preferably not higher than 2 ml/l, more preferably not higher than 0.5 ml/l. It is most preferred that no benzyl alcohol is contained in the developing solutions.

Preferably, the developing solutions of the present invention contain substantially no sulfite. This is because sulfite ion functions as a preservative and at the same time, the sulfite ion has an effect of dissolving the silver halide and reacts with the oxidant of the developing solution to thereby reduce the color forming efficiency. It is presumed that an increase in the fluctuation of photographic characteristics in continuous processing is caused by these effects. The term "containing substantially no sulfite ion" as used herein means that the concentration of sulfite ion is preferably not higher than  $3.0 \times 10^{-3}$  mol/l. It is most preferred that no sulfite ion is contained in the developing solutions. In the present invention, there is included a very small amount of sulfite ion which is used to prevent the processing agent kit from being oxidized (the developing agent is concentrated in the processing agent kit before the preparation of the developing solution).

Preferably, the developing solutions of the present invention contain substantially no sulfite ion. It is also preferred that the developing solutions contain substantially no hydroxylamine. This is because hydroxylamine functions as a preservative. Hydroxylamine itself has silver development activity and photographic characteristics are greatly affected by a fluctuation in the concentration of hydroxylamine. The term "containing substantially no hydroxylamine" as used herein means that the concentration of hydroxylamine is preferably not higher than  $5.0 \times 10^{-3}$  mol/l. It is most preferred that no hydroxylamine is contained in the developing solutions.

It is preferred that the developing solutions of the present invention contain organic preservative in place of hydroxylamine and sulfite ion.

The term "organic preservative" as used herein refers to all organic compounds which reduce the deterioration rate of the aromatic primary amine color developing agents when the organic compounds are added to processing solutions for color photographic materials. Namely, they are organic compounds capable of preventing the color developing agents from being oxidized by air. Particularly effective organic preservatives are hydroxylamine derivatives (excluding hydroxylamine, the same applies hereinbelow), hydroxamic acids, hydrazines, hydrazides, phenols,  $\alpha$ -hydroxyketones,  $\alpha$ -aminoketones, saccharide, monoamines, diamines, polyamines, quaternary ammonium salts, nitroxyl radicals, alcohols, oximes, diamide compounds and condensed cyclic amines. These compounds are described in Japanese Patent Application Nos. 61-147823, 61-173596, 61-165621, 61-188619, 61-197760, 61-186561, 61-198987, 61-201861, 61-186559, 61-170756, 61-188742 and 61-188741, U.S. Pat. Nos. 3,615,503 and

2,494,903, JP-A-52-143020 and JP-B-48-30496 (the term "JP-B" as used herein means an "examined Japanese patent publication").

Substances such as the various metals described in 5 JP-A-57-44148 and JP-A-57-53749, the salicylic acids disclosed in JP-A-59-180588, the alkanolamines disclosed in JP-A-54-3532, the polyethyleneimines disclosed in JP-A-56-94349 and the polyhydroxy compounds disclosed in U.S. Pat. No. 3,746,544 may also be 10 added as other preservatives if required. Addition of an alkanolamine such as triethanolamine, a dialkylhydroxylamine such as diethylhydroxylamine and an aromatic polyhydroxy compound is particularly desirable.

The coating weight (in terms of silver) in the silver 15 halide photographic materials of the present invention is preferably not more than 0.75 g/m<sup>2</sup>, more preferably not more than 0.65 g/m<sup>2</sup>, particularly preferably not more than 0.60 g/m<sup>2</sup>. When the coating weight in terms of silver is more than 0.75 g/m<sup>2</sup>, photographic characteristics 20 greatly fluctuate during continuous processing and the amount of silver left behind is large. Thus, such large coating weight is not preferred for the purpose of the present invention.

Preferably the color developing solutions of the present invention contain chlorine ion in an amount of 25  $3.5 \times 10^{-2}$  to  $1.5 \times 10^{-1}$  mol/l, particularly  $4 \times 10^{-2}$  to  $1 \times 10^{-1}$  mol/l. When the concentration of chlorine ion is higher than  $1.5 \times 10^{-1}$  mol/l, development is retarded. Thus, such a high concentration is not preferred for the purposes of conducting rapid development and providing high maximum density. On the other hand, when the concentration is lower than  $3.5 \times 10^{-2}$  mol/l, fogging by pressure is not sufficiently prevented.

Furthermore, it is also preferred that the color developing solutions of the present invention contain bromine ion in an amount of  $3.0 \times 10^{-5}$  to  $1.0 \times 10^{-3}$  mol/l, particularly  $5.0 \times 10^{-5}$  to  $5 \times 10^{-4}$  mol/l. When the concentration of bromine ion is higher than  $1 \times 10^{-3}$  mol/l, the development is retarded and maximum density and sensitivity are lowered, whereas when the concentration is lower than  $3.0 \times 10^{-5}$  mol/l, fogging by pressure is not sufficiently prevented.

Chlorine ion and bromine ion may be added directly to the developing solutions, or they may be dissolved from the photographic materials into the developing solutions during the course of processing.

When chlorine ion is added directly to color developing solutions, examples of chlorine ion donating materials include sodium chloride, potassium chloride, ammonium chloride, lithium chloride, nickel chloride, magnesium chloride, manganese chloride, calcium chloride and cadmium chloride. Among them, sodium chloride and potassium chloride are preferred.

Chlorine ion may be supplied from fluorescent brightener incorporated in the developing solutions.

Examples of bromine ion-donating materials include sodium bromide, potassium bromide, ammonium bromide, lithium bromide, calcium bromide, magnesium bromide, manganese bromide, nickel bromide, cadmium bromide, cerium bromide and thallium bromide. Among them, potassium bromide and sodium bromide are preferred.

When chlorine ion and bromine ion are dissolved from the photographic materials into the developing solutions, chlorine ion and bromine ion may be supplied from emulsions or from other supply sources.

The pH of the color developing solution used in the invention is preferably 9 to 12 and more preferably 9 to

11.0. The solution may also contain other compounds that constitute known developing solution components.

Preferably, use is made of a buffering agent in order to maintain the abovenoted pH. Examples of buffering agents that may be used include carbonates, phosphates, borates, tetraborates, hydroxybenzoates, glycine salts, N,N-dimethylglycine salts, leucine salts, norleucine salts, guanine salts, 3,4-dihydroxyphenylalanine salts, alanine salts, aminobutyrates, 2-amino 2-methyl-1,3-propanediol salts, valine salts, proline salts, trishydroxyaminomethane salts and lysine salts. Carbonates, phosphates, tetraborates, and hydroxybenzoates in particular have the advantages that they possess excellent solubility and buffering capability in the high pH region of 9.0 or more, they have no adverse effects (fogging, etc.) on photographic performance when they are added to color developing solutions and they are low-cost and the use of these buffering agents is therefore especially preferred.

Specific examples of buffering agents that may be cited include sodium carbonate, potassium carbonate, sodium bicarbonate, potassium bicarbonate, trisodium phosphate, tripotassium phosphate, disodium phosphate, dipotassium phosphate, sodium borate, potassium borate, sodium tetraborate (borax), potassium tetraborate, sodium o-hydroxybenzoate (sodium salicylate), potassium o-hydroxybenzoate, sodium 5-sulfo-2-hydroxybenzoate (sodium 5-sulfosalicylate) and potassium 5-sulfo-2-hydroxybenzoate (potassium 5-sulfosalicylate). However, the invention is not limited to these compounds.

The amount of buffering agent added to the color developing solution is preferably 0.1 mol/l or more, and a particularly preferred amount is 0.1 to 0.4 mol/l.

In addition, various chelating agents may be used in the color developing solution such as calcium and magnesium precipitation preventive agents or agents to improve stability of the solution.

Examples of such nitrilotriacetic acid, diethylenetriaminepentaacetic acid, ethylenediaminetetraacetic acid, N,N,N'-trimethylenephosphonic acid, ethylenediamine-N,N,N',N'-tetramethylenephosphonic acid, transcyclohexanediinetetraacetic acid, 1,2-diaminopropanetetraacetic acid, glycol ether diaminetetraacetic acid, ethylenediamineorthohydroxyphenylacetic acid, 2-phosphonobutane-1,2,4-tricarboxylic acid, 1-hydroxyethylidene-1,1-diphosphonic acid and N,N'-bis(2-hydroxybenzyl)ethylenediamine-N,N'-diacetic acid.

The joint use of two or more of these chelating agents may be made if required.

A suitable amount of such chelating agents to be added is an amount sufficient to block the metal ions in the color developing solution and the amount is, for example, around 0.1 to 10 g per 1 liter.

Any development accelerator may be added to the color developing solution as required. A typical development accelerator that can be used is benzyl alcohol. However, from the point of view of environmental pollution, the solution preparation characteristics and the prevention of color stains, it is preferable that the color developing solution of the invention contain essentially no benzyl alcohol. What is meant by the phrase "essentially" is that there is no more than 2 ml per 1 liter of developing solution and preferably no benzyl alcohol at all is present. Examples of other development accelerators include the thioether compounds disclosed in JP-B-37-16088, JP-B-37-5987, JP-B-38-7826, JP-B-44-12380 and JP-B-45-9019 and U.S. Pat. No. 3,813,247,

etc., the p-phenylenediamine compounds disclosed in JP-A-52-49829 and JP-A-50-15554, the quaternary ammonium salts disclosed in JP-A-50-137726, JP-B-44-30074, JP-A-56-156826 and JP-A-52-43429 etc., the amine compounds disclosed in U.S. Pat. Nos. 2,494,903, 3,128,182, 4,230,796 and 3,253,919, JP-B-41-11431, U.S. Pat. Nos. 2,482,546, 2,596,926 and 3,582,346, etc. and the polyalkylene oxides disclosed in JP-B-37-16088, JP-B-42-25201, U.S. Pat. No. 3,128,183, JP-B-41-11431, JP-B-42-23883 and U.S. Pat. No. 3,532,501, etc., in addition to which 1-phenyl-3-pyrazolidones or imidazoles may be added if required.

In the present invention, any antifoggant may be added if required. Examples of antifoggants that can be used include alkali metal halides such as sodium chloride, potassium bromide or potassium iodide and organic antifoggants. Representative examples of organic antifoggants that may be cited include benzotriazole, 6-nitrobenzimidazole, 5-nitroisoindazole, 5-methylbenzotriazole, 5-nitrobenzotriazole, 5-chlorobenzotriazole, 2-thiazolylbenzimidazole, 2-thiazolylmethylbenzimidazole, indazole, hydroxyazaindolidine, adenine and similar nitrogen-containing heterocyclic compounds.

Brightening agents may be included in the color developing solution that is used in the present invention. 4,4'-diamino-2,2'-disulfostilbene compounds are preferred as brightening agents. The amount to be added is 0 to 5 g/l and preferably 0.1 to 4 g/l.

Also, various surfactants such as alkylsulfonic acids, arylphosphonic acids, aliphatic carboxylic acids and aromatic carboxylic acids may be added if required.

The processing temperature of the color developing solution of the invention is 20° to 50° C. and preferably 30° to 40° C. The processing time is 20 seconds to 5 minutes and preferably 30 seconds to 2 minutes. The amount of replenishment is preferably on the low side and is 20 to 600 ml and preferably 50 to 300 ml per 1 m<sup>2</sup> of the photographic material. 60 to 200 ml is even more preferable and 60 to 150 ml is the most preferable amount.

Next, the desilvering process in the invention will be described. Generally, it is satisfactory if a process containing a bleaching step-fixing step, a fixing step-bleach-fixing step, a bleaching step-bleach-fixing step or a bleach-fixing step is used for the desilvering process.

There now follows a description of the bleaching solutions, bleach-fixing solutions and the fixing solutions that are employable in the invention.

Any bleaching agent may be used in the bleaching solution or in the bleach-fixing solution of the invention but materials such as organic ferric (III) complex salts (e.g., complex salts of aminopolycarboxylic acids such as ethylenediaminetetraacetic acid, diethylenetriaminepentaacetic acid, aminopolyphosphonic acids, phosphonocarboxylic acids and organic phosphonic acids), organic acids such as citric acid, tartaric acid and malic acid, etc., persulfates and hydrogen peroxide are preferred.

Among these materials, organic ferric(III) complex salts are particularly preferable from the point of view of speed of processing and prevention of environmental pollution. Examples that can be given include aminopolycarboxylic acids, aminopolyphosphonic acids, organic phosphonic acids and salts thereof that are useful for forming organic ferric (III) complex salts are ethylenediaminetetraacetic acid, diethylenetriaminepentaacetic acid, 1,3-diaminopropanetetraacetic

acid, propylenediaminetetraacetic acid, nitrilotriacetic acid, cyclohexanediaminetetraacetic acid, methyliminodiacetic acid, iminodiacetic acid and glycol ether diaminetetraacetic acid. These compounds may be in the form of sodium, potassium, lithium or ammonium salts. Among the compounds, ferric (III) complex salts of ethylenediaminetetraacetic acid, diethylenetriamine-pentaacetic acid, cyclohexanediaminetetraacetic acid, 1,3-diaminopropanetetraacetic acid and methyliminodiacetic acid are particularly preferred since they have high bleaching power. These ferric ion complex salts, may be used in the form of complex salts or ferric ion complex salts may be formed in solution using a ferric salt, e.g., ferric sulfate, ferric chloride, ferric nitrate, ferric ammoniumsulfate or ferric phosphate, and a chelating agent such as an aminopolycarboxylic acid, aminopolypophosphonic acid or phosphonocarboxylic acid. Also, the chelating agent may be used in an amount that is in excess of the amount needed for forming a ferric ion complex salt. Among iron complexes, aminopolycarboxylic acid iron complexes are preferred and the amount thereof which may be added is preferably 0.01 to 1.0 mol/l and more preferably 0.05 to 0.50 mol/l.

A variety of compounds may be employed as bleaching accelerators in the bleaching solution, bleach-fixing solution or in their prebaths. Materials that are suitable because they have excellent bleaching power are, e.g., the compounds possessing mercapto groups or disulfide bonds that are disclosed in the Specification of U.S. Pat. No. 3,893,858, the Specification of German Patent 1,290,812, JP-A-53-95630 and *Research Disclosure*, Volume 17129 (July 1978) and thiourea compounds and iodine and bromine ions and other halogen compounds disclosed in JP-B-45-8506, JP-A-52-20832, JP-A-53-32735 and U.S. Pat. No. 3,706,561.

In addition, the bleaching solution or bleach-fixing solution used in the invention may also contain a rehalogenation agent such as a bromide (e.g., potassium bromide, sodium bromide, ammonium bromide), a chloride (e.g., potassium chloride, sodium chloride, ammonium chloride) or an iodide (e.g., ammonium iodide). If required, one or more inorganic or organic acids or alkali metal or ammonium salts thereof with pH buffering capabilities such as borax, sodium metaborate, acetic acid, sodium acetate, sodium carbonate, potassium carbonate, phosphorous acid, phosphoric acid, sodium phosphate, citric acid, sodium citrate and tartaric acid and corrosion preventives such as ammonium nitrate and guanidine may be added.

The fixing agents used in the bleach-fixing solution or fixing solution according to the invention are known fixing agents, i.e., water-soluble silver halide solvents such as sodium thiosulfate, ammonium thiosulfate and similar thiosulfates; sodium thiocyanate, ammonium thiocyanate and similar thiocyanates; ethylenebisthio-glycolic acid, 3,6-dithia-1,8-octane diol and similar thioether compounds and thioureas. One or a mixture of two or more of these substances may be used. It is also possible to use, for example, special bleach-fixing solutions containing combinations of a large amount of a halide such as potassium iodide and the fixing agents disclosed in JP-A-55-155354. In the invention, the use of thiosulfates, especially ammonium thiosulfate is preferred. The amount of fixing agent per 1 liter is preferably 0.3 to 2 moles and is more preferably in the range of 0.5 to 1.0 mole. The pH region of the bleach-fixing

solution or the fixing solution is preferably 3 to 10 and more preferably is 5 to 9.

In addition, various brightening agents, antifoaming agents, surfactants, organic solvents such as methanol, and polyvinylpyrrolidone, etc. may be included in the bleach-fixing solution.

A preservative in the form of a sulfite ion releasing compound such as a sulfite (e.g., sodium sulfite, potassium sulfite, ammonium sulfite), a bisulfite (e.g., ammonium bisulfite, sodium bisulfite, potassium bisulfite) or a metabisulfite (e.g., potassium metabisulfite, sodium metabisulfite, ammonium metabisulfite) may be included in the bleach-fixing solution or fixing solution in the invention. Converted to sulfite ions, the amount of such compounds included is preferably 0.02 to 0.05 mol/l and is more preferably 0.04 to 0.40 mol/l.

Normally, sulfites are added as preservatives but one may also add substances such as ascorbic acid, carbonyl bisulfite adducts and carbonyl compounds.

Further, brightening agents, chelating agents, anti-foaming agents and mold preventives may be added if required.

Generally, the silver halide color photographic light-sensitive material of the invention is washed with water and/or given a stabilization treatment after the desilvering treatment comprising fixing or bleachfixing, etc.

The amount of water in the washing stage or step can be set over a wide range depending on the characteristics of the photographic material (which depends on, e.g., the materials used as couplers, etc.), the intended use and a variety of conditions such as the temperature of the washing water, the number of washing tanks (the number of stages) and whether the replenishment system is a counter-flow or a direct flow system, etc. Among these various factors, the relationship between the amount of water and the number of washing tanks in a multistage counter-flow system can be determined by the method described in the Journal of the Society of Motion Picture and Television Engineers, Vol. 64, p. 248 to 253 (May 1955 number). Normally, the number of stages in a multistage counterflow system is preferably 2 to 6, 2 to 4 being particularly preferred.

A multistage counterflow system permits considerable reduction of the amount of washing water, which can be made, for instance, less than 0.5 to 1 liter per 1 m<sup>2</sup> of photographic material. However, although the advantages of the invention are very marked there can be problems such as the proliferation of bacteria and adhesion of suspended matter to the photographic material as the in-tank dwell time of the water increases. A very effective measure which can be employed for resolving such problems during processing of the photosensitive material of the invention is the method of reducing calcium and magnesium described in JP-A-62-288838. One can also make use of the isothiazolone compounds and the thiabendazole compounds disclosed in JP-A-57-8542, the chlorinated sodium isocyanurate and other chlorinated bactericides disclosed in JP-A-61-120145, the benzotriazoles described in JP-A-61-267761, copper ions and other bactericides such as described in "Antibacterial, Antimold Chemistry" by Hiroshi Horiguchi, "Microorganism Disinfection, Bactericidal, Antimold Technology" edited by the Eisei Gijutsukai (Hygiene Technology Society) and the "Dictionary of Antibacterial Antimold Agents" edited by the Nihon Bokinbobai Gakkai (Japan Bacteria/Mold Prevention Institute).

The washing water may also contain a surfactant as a draining agent and a chelating agent, typically EDTA, as a hard water softener.

Moreover, it is also possible to effect treatment in a stabilization solution following the washing stage or to effect this treatment without going through a washing stage. A stabilization solution contains compounds having the ability to stabilize the image. Examples of such compounds include aldehydes as typified by formalin, buffering agents for adjusting the pH of the film to a value suitable for dye stabilization and ammonium compounds. It is also possible to use the various abovenoted bactericides and antimold agents in the solution in order to prevent proliferation of bacteria and impart mold resistance to the photosensitive material after processing.

In addition, surfactants, brightening agents and hardeners may also be added. Any known method such as disclosed in, for example, JP-A-57-8543, JP-A-58-14834 and JP-A-60-220345 may be employed if stabilization is effected directly without going through a washing stage in the processing of the photographic material of the invention.

Another suitable procedure is to use 1-hydroxyethylidene-1,1-diphosphonic acid, ethylenediaminetetramethyleneephosphonic acid or a similar chelating agent and magnesium or bismuth compounds.

Similarly, a so-called rinse solution may also be used as the stabilization solution or the washing solution that is used after the desilvering treatment in the invention.

The pH in the washing or the stabilization stage in the invention is preferably 4 to 10 and more preferably is 5 to 8. The temperature can be set to a variety of values depending on the intended use and characteristics, etc. of the photographic material but generally it is preferably 15° to 45° C. and more preferably it is 20° to 40° C. The time can be set to any duration but a short duration is desirable from the point of view of reducing the processing time and preferably the time is 15 seconds to 1 minute 45 seconds or more preferably 30 seconds to 1 minute 30 seconds. From the point of view of aspects such as running costs, reduction of the amount of discharged material and handling, the amount of replenishment is preferably kept low.

A specifically preferred replenishment quantity per unit area of the photographic material is 0.5 to 50 times and preferably 3 to 40 times the amount carried in from the prebath, or not more than 1 liter and preferably not more than 500 ml per 1 m<sup>2</sup> of the photographic material. Replenishment may be conducted continuously or intermittently.

The solutions used in the washing and/or stabilization stage can also be used in the preceding stage. An example is the reduction of the amount of waste solution by a multistage counterflow system in which reduced washing water overflow is forced to run into the preceding bleach-fixing bath and a supplementary supply of concentrated solution is supplied into this bath.

The total of the desilvering stage and the washing and the stabilization stage times preferably is not more than 2 minutes and more preferably is 30 seconds to 1 minute 30 seconds. What is meant by the total time is the time from when the silver halide color photographic light-sensitive material comes into contact with the first bath in the desilvering stage to when it exits from the last bath of the washing or the stabilization stage and it includes the waste time for intermediate transport.

What is meant by the statement that the sum of the desilvering treatment and the washing and the stabilization treatment times is not more than 2 minutes is that the sum of the times required for the desilvering treatment and the treatment effected up to the drying stage (more specifically the washing and/or stabilizing stage) is not more than 2 minutes. For example, the sum for the processes such as

- (1) desilvering → Washing
  - (2) desilvering → stabilization
  - (3) desilvering → washing stabilization
- is not more than 2 minutes.

#### EXAMPLE 1

A silver halide emulsion (1) was prepared in the following manner:

|                                                                                                                                                   |         |
|---------------------------------------------------------------------------------------------------------------------------------------------------|---------|
| <u>Solution 1:</u>                                                                                                                                |         |
| H <sub>2</sub> O                                                                                                                                  | 1000 ml |
| NaCl                                                                                                                                              | 3.3 g   |
| Gelatin                                                                                                                                           | 32 g    |
| <u>Solution 2:</u>                                                                                                                                |         |
| Sulfuric acid (1N)                                                                                                                                | 24 ml   |
| <u>Solution 3:</u>                                                                                                                                |         |
| The following compound A (1% aqueous solution)                                                                                                    | 3 ml    |
| $  \begin{array}{c}  \text{CH}_3 \\    \\  \text{N} \\  \text{---} \\  \text{C}=\text{S} \\    \\  \text{N} \\    \\  \text{CH}_3  \end{array}  $ |         |
| <u>Solution 4:</u>                                                                                                                                |         |
| NaCl                                                                                                                                              | 9.9 g   |
| KBr                                                                                                                                               | 2.2 g   |
| Add H <sub>2</sub> O to make                                                                                                                      | 200 ml  |
| <u>Solution 5:</u>                                                                                                                                |         |
| AgNO <sub>3</sub>                                                                                                                                 | 32.00 g |
| Add H <sub>2</sub> O to make                                                                                                                      | 200 ml  |
| <u>Solution 6:</u>                                                                                                                                |         |
| NaCl                                                                                                                                              | 39.6 g  |
| KBr                                                                                                                                               | 9.0 g   |
| Add H <sub>2</sub> O to make                                                                                                                      | 560 ml  |
| <u>Solution 7:</u>                                                                                                                                |         |
| AgNO <sub>3</sub>                                                                                                                                 | 128 g   |
| Add H <sub>2</sub> O to make                                                                                                                      | 560 ml  |

Solution 1 was heated to 54° C. Solution 2 and solution 3 were added thereto. Subsequently, solution 4 and solution 5 were simultaneously added thereto over a period of 14 minutes. After 10 minutes, solution 6 and solution 7 were simultaneously added thereto over a period of 15 minutes. After 5 minutes, the temperature was lowered and the mixture was desalted.

Water and gelatin for dispersion were added thereto and the pH of the mixture was adjusted to 6.2, thus obtaining a monodisperse cubic silver chlorobromide emulsion having a mean grain size of 0.48 μm and a coefficient of variation (a value s/d obtained by dividing the standard deviation by the mean grain size) of 0.10. Sodium thiosulfate was added to the emulsion at 58° C. and chemical sensitization was suitably carried out so as to give a surface latent image type emulsion.

In the same manner as that described above, emulsions (2) to (9) shown in Table 1 were prepared. Emulsions (5) to (8) were prepared according to the method that before chemical sensitization was conducted in the

presence of sodium thiosulfate,  $4.0 \times 10^{-4}$  mol (per mol of silver halide) of the following compound B was added, 1 mol % (based on the amount of silver) of ultra-fine silver bromide grain emulsion (having a grain size of  $0.05\mu$ ) was then added and ripening was carried out at  $58^\circ\text{C}$ . for 10 minutes.

It was found by X-ray diffractometry, by the electron microscope and by the EDX method that emulsions (5) to (8) had silver bromide localized phases having a silver bromide content of not higher than 60 mol % in the vicinity of the apexes of the grains.

The addition of metal ion to emulsions (2) to (4) and emulsions (6) to (9) was made by mixing each of potassium hexachloroiridate(III), potassium hexachlororhodate and potassium ferrocyanide in the form of an aqueous solution with solution 6 and adding each solution.



TABLE 1

| Emulsion No. | Cl Content (nmol %) | Size ( $\mu\text{m}$ ) | Coefficient of Variation | Metal Ion Species | Amount of Added Metal Ion (mol/mol of Ag) |
|--------------|---------------------|------------------------|--------------------------|-------------------|-------------------------------------------|
| 1            | 99                  | 0.48                   | 0.10                     | —                 | —                                         |
| 2            | 99                  | 0.48                   | 0.10                     | iridium           | $5 \times 10^{-8}$                        |
| 3            | 99                  | 0.48                   | 0.10                     | rhodium           | $1 \times 10^{-8}$                        |
| 4            | 99                  | 0.48                   | 0.10                     | iron              | $1 \times 10^{-8}$                        |
| 5            | 99*                 | 0.48                   | 0.10                     | —                 | —                                         |
| 6            | 99*                 | 0.48                   | 0.10                     | iridium           | $5 \times 10^{-8}$                        |
| 7            | 99*                 | 0.48                   | 0.10                     | rhodium           | $1 \times 10^{-8}$                        |
| 8            | 99*                 | 0.48                   | 0.10                     | iron              | $1 \times 10^{-8}$                        |
| 9            | 99                  | 1.01                   | 0.10                     | iridium           | $5 \times 10^{-8}$                        |

\*Emulsions had silver bromide localized phases having a silver bromide content of 60 mol % in the vicinity of the apexes of the grains.

Both sides of a paper support were laminated with polyethylene. The surface of the laminated paper support was coated with the emulsions to prepare a multi-layer color photographic paper having the following layer structure. The resulting photographic paper was referred to as Sample A. Coating solutions were prepared in the following manner.

#### Preparation of coating solution for first layer

60.0 g of yellow coupler (ExY) and 28.0 g of anti-fading agent (Cpd-1) were dissolved in 150 ml of ethyl acetate, 1.0 ml of solvent (Solv-3) and 3.0 ml of solvent (Solv-4). The resulting solution was added to 450 ml of a 10% aqueous gelating solution containing sodium dodecylbenzenesulfonate and the mixture was dispersed by means of an ultrasonic homogenizer. The resulting dispersion was dissolved in 420 g of emulsion No. 9 of Table 1, which contained the following blue-sensitive sensitizing dye to prepare a coating solution for the first layer. In the same manner as in the preparation of the coating solution for the first layer, coating solutions for the second to the seventh layers were prepared. As the hardener for gelatin, 1,2-bis-(vinylsulfonyl)propane was used for each layer.

The following spectral sensitizing dyes were used.

Blue-sensitive Emulsion Layer:

Anhydro-5,5'-dichloro-3,3'-disulfoethoxythiacyanine hydroxide

Green-sensitive Emulsion Layer:

Anhydro-9-ethyl-5,5'-diphenyl-3,3'-disulfoethoxythiacyanine hydroxide

Red-sensitive Emulsion Layer:

3,3'-Diethyl-5-methoxy-9,9'-(2,2'-dimethyl-1,3-propano)thiacyanine iodide

The following mixture of A;B;C=7:2:1 by mol was used as a stabilizer for each emulsion layer.

A: 1-(2-Acetamino-phenyl)-5-mercaptopotetrazole

B: 1-Phenyl-5 mercaptotetrazole

C: 1-(p-Methoxyphenyl)-5-mercaptopotetrazole

The following compounds were used as irradiation-preventing dyes.

[3-Carboxy-5-hydroxy-4-(3-carboxy-5-oxo-1-(2,5-disul-

Compound B

fonatophenyl)-2-pyrazoline-4-ylidene)-1-propenyl-1-pyrazolyl]benzene-2,5-disulfonate disodium salt.

30 N,N-(4,8-Dihydroxy-9,10-dioxo-3,7-disulfonatoanthracene-1,5-diy)bis(aminomethanesulfonate) tetratosodium salt.

[3-Cyano-5-hydroxy-4-(3-(3-cyano-5-oxo-1-(4-sulfonatophenyl)-2-pyrazoline-4-ylidene)-1-pentanyl)-1-pyrazolyl]benzene-4-sulfonate sodium salt

Layer Structure

35 Each layer had the following composition. Numerals represent coating weight ( $\text{g}/\text{m}^2$ ). The amounts of silver halide emulsions are represented by coating weight in terms of silver.

40 Support

Paper support (both sides thereof were laminated with polyethylene)

#### First Layer: Blue-sensitive layer

45 Silver halide emulsion (No. 9) 0.29

Gelatin 1.80

Yellow coupler (ExY) 0.60

Anti-fading inhibitor (Cpd-1) 0.28

Solvent (Solv-3) 0.01

Solvent (Solv-4) 0.03

#### Second Layer: Color mixing inhibiting layer

Gelatin 0.80

Color mixing inhibitor (Cpd-2) 0.055

Solvent (Solv-1) 0.03

Solvent (Solv-2) 0.015

#### Third Layer: Green-sensitive layer

Silver halide emulsion (No. 1) 0.305

Gelatin 1.40

Magenta coupler (ExM) 0.67

Anti-fading agent (Cpd-3) 0.23

Anti-fading agent (Cpd-4) 0.11

Solvent (Solv-1) 0.20

Solvent (Solv-2) 0.02

#### Fourth Layer: Color mixing inhibiting layer

Gelatin 1.70

Color mixing inhibitor (Cpd-2) 0.065

Ultraviolet light absorber (UV-1) 0.45

Ultraviolet light absorber (UV-2) 0.23

Solvent (Solv-1) 0.05

Solvent (Solv-2) 0.05

#### Fifth Layer: Red-sensitive layer

-continued

|                                                       |      |
|-------------------------------------------------------|------|
| Silver halide emulsion (No. 2)                        | 0.21 |
| Gelatin                                               | 1.80 |
| Cyan coupler (ExC-1)                                  | 0.26 |
| Cyan coupler (ExC-2)                                  | 0.12 |
| Anti-fading inhibitor (Cpd-1)                         | 0.20 |
| <u>Color forming accelerator (Cpd-5)</u>              |      |
| Solvent (Solv-1)                                      | 0.16 |
| Solvent (Solv-2)                                      | 0.09 |
| <u>Sixth Layer: Ultraviolet light absorbing layer</u> |      |
| Gelatin                                               | 0.70 |
| Ultraviolet light absorber (UV-1)                     | 0.26 |
| Ultraviolet light absorber (UV-2)                     | 0.07 |
| Solvent (Solv-1)                                      | 0.30 |
| Solvent (Solv-2)                                      | 0.09 |
| <u>Seventh Layer: Protective layer</u>                |      |
| Gelatin                                               | 1.07 |

- (ExY) Yellow Coupler  
 $\alpha$ -Pivalyl- $\alpha$ -(3-benzyl-1-hydantoinyl)-2-chloro-5-[ $\beta$ -(dodecylsulfonyl)butylamido]acetanilide  
(ExM) Magenta Coupler  
1-(2,4,6-Trichlorophenyl)-3-[2-chloro-5-(3-octadecenylsuccinimido)anilino]-5-pyrazolone  
(ExC-1) Cyan Coupler  
2-Pentafluorobenzamido-4-chloro-5-[2-(2,4-di-tert-amylphenoxy)-3-methylbutylamidophenol  
(ExC-2) Cyan coupler  
2,4-Dichloro-3-methyl-6-[ $\alpha$ -(2,4-di-tert-amylphenoxy)-butylamido]phenol  
(Cpd-1) Anti-fading Agent  
2,5-Di-tert-amylphenyl-3,5-di-tert-butylhydroxybenzoate  
(Cpd-2) Color Mixing Inhibitor  
2,5-Di-tert-octylhydroquinone  
(Cpd-3) Anti-fading agent  
1,4-Di-tert-amyl-2,5-di-octyloxybenzene  
(Cpd-4) Anti-fading Agent  
2,2'-Methylenebis(4-methyl-6-tert-butylphenol)  
(Cpd-5) Color Forming Accelerator  
p-(p-Toluenesulfonamido)-phenyl-dodecane  
(UV-1) Ultraviolet Light Absorber  
2-(2-Hydroxy-3,5-di-tert-amylphenyl)benzotriazole  
(UV-2) Ultraviolet Light Absorber  
2-(2-Hydroxy-3,5-di-tert-butylphenyl)benzotriazole  
(Solv-1) Solvent  
Di(2-ethylhexyl) phthalate  
(Solv-2) Solvent  
Dibutyl phthalate  
(Solv-3) Solvent  
Di(iso-nonyl) phthalate  
(Solv-4) Solvent  
N,N-Diethylcarbonamidomethoxy-2,4-di-t-amylbenzene

Further, the emulsions of the first layer, the third layer and the fifth layer were replaced by the emulsions given in Table 2 to prepare Samples B to H. The dry film thickness of each sample was 10  $\mu$ m and the wet film thickness of each sample was 26  $\mu$ m.

The magenta coupler in the third layer of each of the samples A to H was replaced by an equimolar amount of the magenta coupler (M-2) of the present invention to prepare Samples A' to H'.

TABLE 2

| Sample No. | Emulsion No. Used for First Layer | Emulsion No. Used for Third Layer | Emulsion No. Used for Fifth Layer |
|------------|-----------------------------------|-----------------------------------|-----------------------------------|
| A          | 9                                 | 1                                 | 2                                 |
| B          | 9                                 | 2                                 | 2                                 |

TABLE 2-continued

| Sample No. | Emulsion No. Used for First Layer | Emulsion No. Used for Third Layer | Emulsion No. Used for Fifth Layer |
|------------|-----------------------------------|-----------------------------------|-----------------------------------|
| 5          | C 9                               | 3                                 | 2                                 |
|            | D 9                               | 4                                 | 2                                 |
|            | E 9                               | 5                                 | 2                                 |
|            | F 9                               | 6                                 | 2                                 |
| 10         | G 9                               | 7                                 | 2                                 |
|            | H 9                               | 8                                 | 2                                 |

The thus-obtained samples A to H and A' to H' were subjected to gradation exposure for sensitometry through a green filter using a sensitometer (color temperature of light source: 3,200K, FWH type manufactured by Fuji Photo Film Co., Ltd.) Exposure time was 1/50 sec. and 30 sec. and the amount of exposure was adjusted so that both were 250 CMS.

After exposure, the following processing steps which comprises a color development step, bleach-fix step and a rinsing step were carried out.

The above photographic materials were exposed through an optical wedge and processed in the following processing steps.

| Processing Steps  | Temperature | Time    |
|-------------------|-------------|---------|
| Color development | 35° C.      | 45 sec. |
| Bleach-fixing     | 30-35° C.   | 45 sec. |
| Rinse (1)         | 30-35° C.   | 20 sec. |
| Rinse (2)         | 30-35° C.   | 20 sec. |
| Rinse (3)         | 30-35° C.   | 20 sec. |
| Rinse (4)         | 30-35° C.   | 30 sec. |
| Drying            | 70-80° C.   | 60 sec. |

35 (A four tank countercurrent system of rinse (4)→(1) was used.)

Each processing solution had the following composition:

| Color Developing Solution                                                      |                 |
|--------------------------------------------------------------------------------|-----------------|
| Water                                                                          | 800 ml          |
| Ethylenediamine-N,N,N',N'-tetra methylenephosphonic acid                       | 1.5 g           |
| Triethanolamine                                                                | 8 g             |
| Sodium chloride                                                                | 1.4 g           |
| Potassium bromide                                                              | 0.004 g         |
| Potassium carbonate                                                            | 25 g            |
| N-Ethyl-N-( $\beta$ -methanesulfonamido-ethyl)-3-methyl-4-aminoaniline sulfate | 5.0 g           |
| N,N-Bis(carboxymethyl)hydrazine                                                | 5.0 g           |
| Fluorescent brightener (UVITEX CK, a product of Ciba-Geigy)                    | 2.0 g           |
| Add water to make pH (25° C.)                                                  | 1000 ml         |
| Bleach-fixing Solution                                                         | 10.10           |
| Water                                                                          | 400 ml          |
| Ammonium thiosulfate (70% aqueous solution)                                    | 100 ml          |
| Sodium sulfite                                                                 | 18 g            |
| Ethylenediaminetetraacetic acid                                                | 55 g            |
| iron (III) ammonium                                                            |                 |
| Disodium ethylenediaminetetraacetate                                           | 3 g             |
| Ammonium bromide                                                               | 40 g            |
| Add water to make pH (25° C.)                                                  | 1000 ml         |
|                                                                                | adjusted to 6.0 |

## Rinsing Water

65 Ion exchanged water (each concentration of calcium and magnesium was 2.5 ppm)

The reflection density of the processed samples was measured and the characteristic curve was prepared.

The reciprocal of the exposure amount giving a density 0.5 higher than the fog density was taken as the sensitivity. Sensitivity obtained by exposing sample A immediately after preparation for 30 seconds and then developing it for 45 seconds was referred to as 100. Other sensitivity was represented by a relative value. The change in sensitivity was examined when the exposure time was varied.

In order to examine the resistance to fluctuation in the processing factors, there was taken, as an index of processing dependence, a value obtained by dividing the sensitivity (when the development time in the above color development was 30 seconds) by the sensitivity (when the development time was 90 seconds) and multiplying the quotient by 100. The exposure time was fixed to 30 seconds.

The results are shown in Table 3.

TABLE 3

| Sample No. | 30 sec. Exposure |                       | 1/50 sec Exposure |                      | Remarks   |
|------------|------------------|-----------------------|-------------------|----------------------|-----------|
|            | Sensitivity      | Processing Stability* | Sensitivity       | Processing Stability |           |
| A          | 100              | 60                    | 48                | 45                   | Comp. Ex. |
| B          | 110              | 63                    | 100               | 51                   |           |
| C          | 80               | 70                    | 90                | 60                   |           |
| D          | 110              | 71                    | 95                | 63                   |           |
| E          | 150              | 62                    | 70                | 49                   |           |
| F          | 165              | 65                    | 155               | 51                   |           |
| G          | 120              | 71                    | 130               | 60                   |           |
| H          | 160              | 73                    | 140               | 62                   |           |
| A'         | 120              | 72                    | 60                | 77                   | Invention |
| B'         | 130              | 89                    | 125               | 88                   |           |
| C'         | 90               | 85                    | 95                | 87                   |           |
| D'         | 120              | 85                    | 110               | 85                   |           |
| E'         | 165              | 73                    | 80                | 74                   | Comp. Ex. |
| G'         | 180              | 90                    | 170               | 89                   | Invention |
| H'         | 130              | 92                    | 140               | 88                   |           |
| H'         | 180              | 89                    | 175               | 86                   |           |

\*The closer the value of processing stability to 100, the higher is the processing stability.

It is apparent from Table 3 that the photographic materials of the present invention highly highly sensitive over a wide illumination intensity range and have a high processing stability.

## EXAMPLE 2

Samples A to H and A' to H' of Example 1 were tested in the same manner as in Example 1 except that the following development processing steps were carried out using the following processing solutions.

It was found that the present invention had similar remarkable effects as in Example 1.

The above photographic materials were exposed through an optical wedge and processed in the following steps:

| Processing Step   | Temperature | Time    |
|-------------------|-------------|---------|
| Color development | 35° C.      | 45 sec. |
| Bleach-fixing     | 30-36° C.   | 45 sec. |
| Stabilization (1) | 30-37° C.   | 20 sec. |
| Stabilization (2) | 30-37° C.   | 20 sec. |
| Stabilization (3) | 30-37° C.   | 20 sec. |
| Stabilization (4) | 30-37° C.   | 30 sec. |
| Drying            | 70-85° C.   | 60 sec. |

A four tank countercurrent system of stabilization (4)→(1) was used.

Each processing solution had the following composition:

| Color Developing Solution                                                     |                 |
|-------------------------------------------------------------------------------|-----------------|
| Water                                                                         | 800 ml          |
| Ethylenediaminetetraacetic acid                                               | 2.0 g           |
| Triethanolamine                                                               | 8.0 g           |
| Sodium chloride                                                               | 1.4 g           |
| Potassium bromide                                                             | 0.004 g         |
| Potassium carbonate                                                           | 25 g            |
| N-Ethyl-N-( $\beta$ -methanesulfonamidoethyl)-3-methyl-4-aminoaniline sulfate | 5.0 g           |
| N,N-Diethylhydroxylamine                                                      | 4.2 g           |
| 5,6-Dihydroxybenzene-1,2,4-trisulfonic acid                                   | 0.3 g           |
| Fluorescent brightener (4,4'-diaminostilbene type)                            | 2.0 g           |
| Add water to make                                                             | 1000 ml         |
| pH (25° C.)                                                                   | 10.10           |
| Bleach-fixing Solution                                                        |                 |
| Water                                                                         | 400 ml          |
| Ammonium thiosulfate (70% aqueous solution)                                   | 100 ml          |
| Sodium sulfite                                                                | 18 g            |
| Ethylenediaminetetraacetic acid                                               | 55 g            |
| iron (III) ammonium                                                           | 3 g             |
| Disodium ethylenediaminetetraacetate                                          | 8 g             |
| Glacial acetic acid                                                           | 1000 ml         |
| Add water to make                                                             | adjusted to 5.5 |
| pH (25° C.)                                                                   |                 |
| Stabilizing Solution                                                          |                 |
| Formalin (37% aqueous solution)                                               | 0.1 g           |
| Formalin-sulfurous acid adduct                                                | 0.7 g           |
| 5-Chloro-2-methyl-4-isothiazoline-3-one                                       | 0.01 g          |
| Copper sulfate                                                                | 0.005 g         |
| Add water to make                                                             | 1000 ml         |
| pH (25° C.)                                                                   | adjusted to 4.0 |

## EXAMPLE 3

Samples F and F' of Example 1 were subjected to the following test to examine the relationship between bromine ion concentration in the developing solution and fog after processing.

## Exposure:

The same way as in Example 1 except that the exposure time was 30 seconds.

## Processing:

#1; the same as in Example 2 except that development time was 90 seconds.

#2; the same as in Example 2 except that the color developing solution contained no potassium bromide and the development time was 90 seconds.

The reflection density of the processed samples was measured and the characteristic curve was prepared. The reciprocal of the amount of exposure giving a density higher by 0.5 than the fog density was taken as the sensitivity. The sensitivity obtained by processing sample F by processing #1 was referred to as 100. Other sensitivity was represented by a relative value. The values of fog density and sensitivity are shown in Table 4.

TABLE 4

| Sample No. | Processing | Fog Density | Sensitivity | Remarks   |
|------------|------------|-------------|-------------|-----------|
| F          | #1         | 0.02        | 100         | Comp. Ex. |
| F          | #2         | 0.03        | 98          | "         |
| F'         | #1         | 0.005       | 110         | Invention |
| F'         | #2         | 0.03        | 107         | Comp. Ex. |

It is apparent from Table 4 that fogging is remarkably decreased when the color photographic material of the

present invention is processed by using a color developing solution containing bromine ion in the range of  $3 \times 10^{-5}$  to  $1.0 \times 10^{-3}$  mol/l.

According to the present invention, there can be provided a color photographic material which can be rapidly processed, is highly sensitive and less fogged over a wide exposure range, is not affected very much by fluctuations in development conditions and is of stable quality.

While the invention has been described in detail and with reference to specific embodiments thereof, it will be apparent to one skilled in the art that various changes and modifications can be made therein without departing from the spirit and scope thereof.

What is claimed is:

1. A silver halide color photographic light-sensitive material, comprising at least one silver halide light-sensitive emulsion layer provided on a support wherein at least one of said light-sensitive emulsion layer contains (i) at least one 5-pyrazolone coupler and (ii) at least one monodisperse cubic silver halide emulsion containing at least an iridium ion in an amount from  $1 \times 10^{-9}$  to  $1 \times 10^{-3}$  mol per mol of silver halide, said emulsion being obtained by incorporating said metal ion into silver halide grains in the silver halide light-sensitive emulsion by adding the ion to an emulsion formation system before or during formation of the grains or after formation of the grains but before the addition of a chemical sensitizer; wherein said 5-pyrazole coupler is represented by the following formulas: represented by the following formulas:



wherein R<sup>1</sup> represents a hydrogen atom, an alkyl group, an aryl group or a heterocyclic group; R<sub>3</sub> is an anilino group, an acylamino group, a ureido group, a carbamoyl group, an alkoxy group, an allyloxycarbonyl group, an alkoxy carbonyl group or an N-heterocyclic group; R<sub>4</sub> is a substituted or unsubstituted aryl group; R<sub>c</sub> and R<sub>d</sub> each represents halogen atoms or a group selected from the group consisting of R<sub>b</sub> and Z<sub>2</sub>R<sub>g</sub>; R<sub>e</sub> is a hydrogen atom or a group as defined for R<sub>c</sub> and R<sub>d</sub>; R<sub>b</sub> is a substituted or an unsubstituted alkyl, aryl or heterocyclic group; Z<sub>2</sub> represents an oxygen atom or a sulfur atom or NR<sub>h</sub>; R<sub>f</sub> is a hydrogen atom or a group as defined for R<sub>b</sub>; R<sub>g</sub> is a group defined for R<sub>f</sub>; R<sub>h</sub> is a group as defined for R<sub>f</sub>; R<sub>c</sub> may bond with R<sub>d</sub> and/or R<sub>e</sub> to form one or two carbon rings or hetero rings and these may also possess substituents; X represents an atomic group required for the formation of a ring; B represents a carbon atom, an oxygen atom, a nitrogen atom or a sulfur atom; i represents 0 or 1;



15 wherein R<sub>1</sub>, R<sub>3</sub>, R<sub>4</sub> and X signify the same atoms, groups and atomic groups as defined above; Y<sub>3</sub> represents a substituent or an unsubstituted methylene or ethylene group or



25 Rf signifies the same atoms and groups as noted as defined above;



wherein R<sub>1</sub>, R<sub>3</sub> and R<sub>4</sub> each signifies the same atoms and groups as defined above; R<sub>6</sub> and R<sub>7</sub> each represents an alkyl group or an aryl group; R<sub>8</sub> represents a substituted or unsubstituted methylene group or a substituted or unsubstituted ethylene group; D represents a methylene group or an oxygen, nitrogen or sulfur atom; n represents an integer from 0 to 2 when it is a methylene group and is 1 in the other cases; and p is an integer from 0 to 3.

50 2. The silver halide color photographic light-sensitive material as in claim 1, wherein the photographic material has a dry film thickness of not more than 15  $\mu\text{m}$  and a wet film thickness from 20 to 40  $\mu\text{m}$ .

3. The silver halide color photographic light sensitive material as in claim 1, wherein said iridium ion is derived from an iridium salt or an iridium complex salt.

4. The silver halide color photographic light-sensitive material as in claim 1, wherein in formula (I), R<sub>1</sub> represents a substituted or an unsubstituted aliphatic group having from 1-22 carbon atoms, a substituted or an unsubstituted aryl group selected from the group consisting of a phenyl group and a naphthyl group, and a substituted or an unsubstituted heterocyclic group selected from the group consisting of a 2-furyl group, a 2-thienyl group, a 2-pyrimidinyl group and a 4-pyridyl group.

5. The silver halide color photographic light-sensitive material as in claim 1, wherein the substituents of said

substituted groups represented by  $R_1$  in said 5-pyrazolone coupler is selected from the group consisting of a halogen atom, an aliphatic group, an aryl group, a heterocyclic group, an alkoxy group, an alkoxy group, an alkylamino group, an alkoxy carbonyl group, a carbamoyl group, an anilino group, a sulfamoyl group, an alkylsulfonyl group, an arylsulfonyl group, an alkylthio group, an arylthio group, an acyl group, an acylamino group, an imido group, a ureido group, a sulfamoylamino group, an alkoxy carbonylamino group, a sulfonamido group, a hydroxyl group and a cyano group.

6. The silver halide color photographic light-sensitive material as in claim 1, wherein said 5-pyrazolone coupler is represented by the following general formula:



wherein  $R_1$ ,  $R_3$ ,  $R_4$ ,  $Rc$ ,  $Rd$ ,  $Re$ ,  $X$ ,  $B$  and  $i$  signify the same atom or groups as defined in claim 1.

7. The silver halide color photographic light-sensitive material as in claim 1, wherein said 5-pyrazolone coupler is represented by the following general formula:



wherein  $R_1$ ,  $R_3$ ,  $R_4$  and  $X$  signify the same atoms, groups and atomic groups as defined in claim 1;  $Y_3$  represents a substituted or an unsubstituted methylene or ethylene group or



$Rf$  signifies the same atoms and groups as defined in claim 1.

8. The silver halide color photographic light-sensitive material as in claim 1, wherein said 5-pyrazolone coupler is represented by the following general formula:



15 wherein  $R_1$ ,  $R_3$  and  $R_4$  each signifies the same atoms and groups as defined in claim 1;  $R_6$  and  $R_7$  each represents an alkyl group or an aryl group;  $R_8$  represents a substituent for  $L_1$  and  $L_2$ ;  $D$  represents a methylene group or an oxygen, nitrogen or sulfur atom;  $n$  represents an integer from 0 to 2 when it is a methylene group and is 1 in the other cases; and  $p$  is an integer from 0 to 3.

20 9. The silver halide color photographic light sensitive material as in claim 8, wherein  $R_8$  is a substituent selected from the group consisting of a halogen atoms, an aliphatic group, an aryl group, a heterocyclic group, an alkoxy group, an aryloxy group, an alkylamino group, an alkoxy carbonyl group, a carbamoyl group, an anilino group, a sulfamoyl group, an alkylsulfonyl group, an arylsulfonyl group, an alkylthio group, an arylthio group, an acyl group, an acylamino group, an imido group, a ureido group, a sulfamoylamino group, an alkoxy carbonylamino group, a sulfonamido group, a hydroxyl group and a cyano group.

25 10. The silver halide color photographic light-sensitive material as in claim 8, wherein  $D$  represents a nitrogen atom which is substituted with hydrogen or with a substituent group.

30 11. The silver halide color photographic light-sensitive material as in claim 1, wherein said 5-pyrazolone magenta coupler is used in an amount of from  $1 \times 10^{-3}$  to 1 mol per mol of silver halide in the silver halide emulsion.

35 12. The silver halide color photographic light-sensitive material as in claim 1, wherein said silver halide comprises silver chloride or silver chlorobromide containing at least 90 mol % of silver chloride.

40 13. The silver halide color photographic light-sensitive material as in claim 1, wherein  $B$  is  $-\text{CH}_2-$ ,  $=\text{CH}-$ , a substituted



45 55 14. The silver halide color photographic light-sensitive material as in claim 1, wherein  $B$  is  $=\text{CH}-$  or a substituted



\* \* \* \* \*